



US006590317B2

(12) **United States Patent**  
Nishikawa et al.

(10) Patent No.: US 6,590,317 B2  
(45) Date of Patent: \*Jul. 8, 2003

(54) SPARK PLUG

(75) Inventors: **Kenichi Nishikawa**, Bisai (JP);  
**Yoshihide Kouge**, Kagoshima (JP);  
**Makoto Sugimoto**, Nagoya (JP)

(73) Assignee: **NGK Spark Plug Co., Ltd., Nagoya**  
(JP)

(\*) Notice: Subject to any disclaimer, the term of this patent is extended or adjusted under 35 U.S.C. 154(b) by 112 days.

This patent is subject to a terminal disclaimer.

(21) Appl. No.: 09/867,759

(22) Filed: **May 31, 2001**

(65) **Prior Publication Data**

US 2002/0036451 A1 Mar. 28, 2002

(30) **Foreign Application Priority Data**

May 31, 2000 (JP) ..... 2000-163846  
Mar. 30, 2001 (JP) ..... 2001-099528

(51) Int. Cl.<sup>7</sup> ..... H01T 13/00; H01T 13/52

(52) U.S. Cl. .... 313/118

(58) **Field of Search** ..... 313/118, 119,  
313/120, 121, 122, 123, 124, 125, 126,  
127, 128, 129, 130, 131 R, 131 A, 132,  
133, 134, 135, 136, 137, 138, 139, 140,  
141, 142, 143, 144, 145; 123/169 EL, 169 R;

(56) **References Cited**

## U.S. PATENT DOCUMENTS

5,109,178 A \* 4/1992 Yoshida et al. .... 313/137  
 6,274,971 B1 \* 8/2001 Sugimoto et al. .... 313/143

## FOREIGN PATENT DOCUMENTS

JP 11-43351 2/1999  
JP 11-106234 4/1999

## OTHER PUBLICATIONS

Nishikawa et al. U.S. patent application Publication 2002/0033659 A1.\*

\* cited by examiner

*Primary Examiner*—Nimeshkumar D. Patel

*Assistant Examiner*—Sharlene Leurig

(74) *Attorney, Agent, or Firm*—Morgan, Lewis & Bockius LLP

(57) **ABSTRACT**

A glaze layer 2d of the spark plug has the composition comprising 1 mol % or less of a Pb component in terms of PbO; 25 to 45 mol % of a Si component in terms of SiO<sub>2</sub>; 20 to 40 mol % of a B component in terms of B<sub>2</sub>O<sub>3</sub>; 5 to 25 mol % of a Zn component in terms of ZnO; 0.5 to 15 mol % of Ba and/or Sr components in terms of BaO or SrO; 5 to 10 mol % in total of at least one alkaline metal component of Na, K and Li in terms of Na<sub>2</sub>O, K<sub>2</sub>O, and Li<sub>2</sub>, respectively, where K is essential; and further, 0.5 to 5 mol % in total of one or two kinds or more of Mo, W, Ni, Co, Fe and Mn in terms of MoO<sub>3</sub>, WO<sub>3</sub>, Ni<sub>3</sub>O<sub>4</sub>, Co<sub>3</sub>O<sub>4</sub>, Fe<sub>2</sub>O<sub>3</sub>, and MnO<sub>2</sub>, respectively.

**34 Claims, 9 Drawing Sheets**



FIG. 1



## FIG. 2



FIG. 3A



FIG. 3B



FIG. 4



## FIG. 5



FIG. 6



## FIG. 7



FIG. 8D



FIG. 8C



FIG. 8B



FIG. 8A



FIG. 9A



FIG. 9B



## 1

## SPARK PLUG

## BACKGROUND OF THE INVENTION

## 1. Field of the Invention

This invention relates to a spark plug.

## 2. Description of the Related Art

A spark plug used for ignition of an internal engine of such as automobiles generally comprises a metal shell to which a ground electrode is fixed, an insulator made of alumina ceramics, and a center electrode which is disposed inside the insulator. The insulator projects from the rear opening of the metal shell in the axial direction. A terminal metal fixture (terminal) is inserted into the projecting part of the insulator and is connected to the center electrode via a conductive glass seal layer which is formed by a glass sealing procedure or a resistor. A high voltage is applied to the terminal metal fixture to cause a spark over the gap between the ground electrode and the center electrode.

Under some combined conditions, for example, at an increased spark plug temperature and an increased environmental humidity, it may happen that high voltage application fails to cause a spark over the gap but, instead, a discharge called as a flashover occurs between the terminal metal fixture and the metal shell, going around the projecting insulator. Primarily for the purpose of avoiding flashover, most of commonly used spark plugs have a glaze layer on the surface of the insulator. The glaze layer also serves to smoothen the insulator surface thereby preventing contamination and to enhance the chemical or mechanical strength of the insulator.

In the case of the alumina insulator for the spark plug, such a glaze of lead silicate glass has conventionally been used where silicate glass is mixed with a relatively large amount of PbO to lower a softening point. In recent years, however, with a globally increasing concern about environmental conservation, glazes containing Pb have been losing acceptance. In the automobile industry, for instance, where spark plugs find a huge demand, it has been a subject of study to phase out Pb glazes in a future, taking into consideration the adverse influences of waste spark plugs on the environment.

Leadless borosilicate glass- or alkaline borosilicate glass-based glazes have been studied as substitutes for the conventional Pb glazes, but they inevitably have inconveniences such as a high glass transition or an insufficient insulation resistance. To address this problem, JP-A-11-43351 proposes a leadless glaze composition having an adjusted Zn component to improve glass stability without increasing viscosity, and JP-A-11-106234 discloses a composition of leadless glaze for improving the insulation resistance by effects of joint addition of alkaline component.

Incidentally, since the glazes for spark plugs are used attaching to engines, they are apt to rise in temperature than cases of general insulating porcelains. Further, in recent years the voltage applied to spark plugs has been increasing together with advancing performance of engines. For these, the glaze for this use has been required to have insulation performance withstanding severer conditions of use. However, the glaze composition disclosed in JP-A-11-106234 is not always satisfactory in insulating performance at high temperatures, particularly the performance as evaluated as a glaze layer formed on an insulator in a spark plug (e.g., anti-flashover properties).

JP-A-11-106234 refers to the improvement of the insulation resistance by effects of joint addition of an alkaline

## 2

component of the glaze containing Si or B as the glass skeleton component, but it could hardly recognized that a satisfactory attention is paid to a cancellation of differential thermal expansion coefficient in relation with the alumina based ceramics as composing ceramics of the insulator, and an improving level of the insulation resistance is not always satisfied.

## SUMMARY OF THE INVENTION

10 It is a first object of the invention to provide such a spark plug having a glaze layer which has a reduced Pb content, is capable of being baked at relatively low temperatures, exhibits excellent insulation properties, and is easy to get a baked smooth surface.

15 It is a second object of the invention to provide such a spark plug where reduced is the differential thermal expansion coefficient in relation with the alumina based ceramics as composing the insulator by adjusting an alkaline metal component in the glaze, thereby to make less to cause defects as cracks or crazing in the glaze layer and farther heighten the insulation resistance.

## BRIEF DESCRIPTION OF THE DRAWINGS

25 FIG. 1 is a whole front and cross sectional view showing the spark plug according to the invention.

FIG. 2 is a front view showing an external appearance of the insulator together with the glaze layer.

30 FIGS. 3A and 3B are vertical cross sectional views showing some examples of the insulator.

FIG. 4 is a whole front view showing another example of the spark plug according to the invention.

35 FIG. 5 is a whole front view showing a further example of the spark plug according to the invention.

FIG. 6 is an explanatory view showing the measuring method of the insulation resistant value of the spark plug.

FIG. 7 is an explanatory view of the forming step of coating the slurry of the glaze.

40 FIGS. 8A to 8D are explanatory views of the gas sealing step.

FIGS. 9A and 9B are explanatory views continuing from FIGS. 8A to 8D.

The reference numerals and sign are set forth below.

1: Metal shell;

2: Insulator;

2d: Glaze layer;

2d': Blaze slurry coated layer;

3: Center electrode;

4: Ground electrode; and

S: Glaze slurry

## DETAILED DESCRIPTION OF THE INVENTION

The spark plug according to the invention comprises an alumina based ceramic insulator disposed between a center electrode and the metal shell, where at least part of the surface of the insulator is covered with a glaze layer comprising oxides.

A first composition thereof is characterized in that the glaze layer comprises 1 mol % or less of Pb component in terms of PbO; 25 to 45 mol % of Si component in terms of SiO<sub>2</sub>; 20 to 40 mol % of B component in terms of B<sub>2</sub>O<sub>3</sub>; 5 to 25 mol % of Zn component in terms of ZnO; 0.5 to 15 mol % of Ba and/or Sr components in terms of BaO or SrO;

at least one alkaline metal components of 5 to 10 mol % in total of Na, K and Li in terms of  $\text{Na}_2\text{O}$ ,  $\text{K}_2\text{O}$ , and  $\text{Li}_2$ , respectively, where K is essential;

and further, one or two kinds or more of Mo, W, Ni, Co, Fe and Mn 0.5 to 5 mol % in total in terms of  $\text{MoO}_3$ ,  $\text{WO}_3$ ,  $\text{Ni}_3\text{O}_4$ ,  $\text{Co}_3\text{O}_4$ ,  $\text{Fe}_2\text{O}_3$ , and  $\text{MnO}_2$ , respectively.

Reference will be hereafter made to effects of the first composition of the inventive spark plug.

(Work & Effect A)

For aiming at the adaptability to the environmental problems, it is a premise that the glaze to be used contains the Pb component 1.0 mol % or less in terms of  $\text{PbO}$  (hereafter called the glaze containing the Pb component reduced to this level as "leadless glaze") When the Pb component is present in the glaze in the form of an ion of lower valency (e.g.,  $\text{Pb}^{2+}$ ), it is oxidized to an ion of higher valency (e.g.,  $\text{Pb}^{3+}$ ) by a corona discharge. If this happens, the insulating properties of the glaze layer are reduced, which probably spoils an anti-flashover. From this viewpoint, too, the limited Pb content is beneficial. A preferred Pb content is 0.1 mol % or less. It is most preferred for the glaze to contain substantially no Pb (except a trace amount of lead unavoidably incorporated from raw materials of the glaze).

(Effect B)

While reducing the Pb content, the glaze used in the invention has a specifically designed composition for securing the insulating properties, optimizing the glaze baking temperature, and improving the finish of the baked glaze face. The Pb component in conventional glazes has played an important role in adjusting a softening point (practically, moderately lowering the softening point of the glaze to secure a fluidity when baking the glaze), and in the leadless glaze, a B component ( $\text{B}_2\text{O}_3$ ) and the alkaline metal component have strong relationship with adjustment of the softening point. Inventors have found that there is a specific range of the B component in relation with a content of the Si component, which is suited to improving of the baking finish, and being based on the premise of this containing range, if one or two kinds or more of Mo, W, Ni, Co, Fe, and Mn are added, it is possible to provide such a spark plug having a glaze layer which can secure the fluidity when baking the glaze, is capable of being fired at relatively low temperatures, exhibits excellent insulation properties, and is easy to get a smooth surface, and thus accomplished this invention. That is, the first problem is solved.

(Effect C)

In the conventional glazes, the Pb component plays an important role as to the fluidity when baking the glaze, but in the leadless glaze of the invention, while containing the alkaline metal component for securing the fluidity when baking the glaze, the high insulating resistance can be provided by determining the containing range of the Si component as above mentioned. That is, the alkaline metal component in the glaze lowers the softening point of the glaze and serves to secure the fluidity when baking the glaze. If containing the alkaline metal component in the above mentioned range, such effects are exhibited which can form the glaze layer difficult to generate pinholes or glaze crimping in an outer appearance.

If the content of the alkaline metal component is less than the above mentioned range, the fluidity when baking the glaze is probably decreased. However, if selecting the total containing amount as above mentioned of the alkaline metal component, it is assumed that such a glaze layer maybe provided which is uniform in thickness and is less to cause glaze crimping or pinholes in the appearance owing to air bubbles involved as glaze slurry.

(Effect D)

Further, the first composition of the invention has a characteristic also in containing essentially K as the alkaline metal component. While securing the fluidity when baking the glaze and in turn improving a smoothness in the glaze layer to be formed, it is possible to largely heighten the insulating performance. The reason therefor is assumed that since the K component has a larger atomic weight than other alkaline metal components of Na and Li in spite of the same mol containing amount and the same cation number, it occupies a larger weight ratio. For more heightening this effect, it is desirable to determine a component of the highest content to be K in the alkaline metal components in the glaze layer.

A second composition of the spark plug according to the invention is characterized in that the glaze layer comprises 1 mol % or less of the Pb component in terms of  $\text{PbO}$ ; 25 to 45 mol % of the Si component in terms of  $\text{SiO}_2$ ; 20 to 40 mol % of the B component in terms of  $\text{B}_2\text{O}_3$ ; 5 to 25 mol % of the Zn component in terms of  $\text{ZnO}$ ; 0.5 to 15 mol % of the Ba and/or Sr components in terms of  $\text{BaO}$  or  $\text{SrO}$ ;

5 to 10 mol % in total of at least one alkaline metal components of Na, K and Li in terms of  $\text{Na}_2\text{O}$ ,  $\text{K}_2\text{O}$  and  $\text{Li}_2$ , respectively;

0.5 to 5 mol % in total of one or two kinds or more of Ti, Zr and Hf in terms of  $\text{TiO}_2$ ,  $\text{ZrO}_2$  and  $\text{HfO}_2$ , respectively, and

0.5 to 5 mol % in total of one or two kinds or more of Mo, W, Ni, Co, Fe and Mn in terms of  $\text{MoO}_3$ ,  $\text{WO}_3$ ,  $\text{Ni}_3\text{O}_4$ ,  $\text{Co}_3\text{O}_4$ ,  $\text{Fe}_2\text{O}_3$ , and  $\text{MnO}_2$ , respectively.

The second structure is the same as the first one in other glaze compositions excepting that the glaze layer does not necessarily take the alkaline metal component K as essential and one or two kinds or more of Ti, Zr and Hf are contained in the above mentioned range. Accordingly, the Effects A to C are similarly accomplished. On the other hand, if containing one or two kinds or more of Ti, Zr and Hf, new effects can be exhibited as follows.

(Effect E)

By addition of Ti, Zr or Hf, a water resistance is improved. As to the Zr or Hf components, the improved effect of the water resistance of the glaze layer is more noticeable. By the way, "the water resistance is good" is meant that if, for example, a powder like raw material of the glaze is mixed together with a solvent as water and is left as a glaze slurry for a long time, such inconvenience is difficult to occur as increasing a viscosity of the glaze slurry owing to elusion of the component. As a result, in case of coating the glaze slurry to the insulator, optimization of a coating thickness is easy and unevenness in thickness is reduced. Subsequently, said optimization and said reduction can be effectively attained. If the addition amount of these components is less than 0.5 mol %, the effect of the optimization is short, probably resulting in lowering of the insulating resistance of the glaze layer by increase of the film thickness.

For the glaze layer, it is possible to select a composition corresponding to the combination of the above first and second ones. Thereby, the Effects A to E can be accomplished at the same time.

A third composition of the spark plug according to the invention is characterized in that the glaze layer comprises 1 mol % or less of the Pb component in terms of  $\text{PbO}$ ; and contains either or both of the Si and B components as a glass skeleton structure, and the glaze layer comprises three components of Li, Na and K as the alkaline metal

components, and has a composition which satisfies the relationship of



where total mol content of  $\text{NLi}_2\text{O}$  of Li component is in terms of  $\text{Li}_2\text{O}$ , mol content of  $\text{NNa}_2\text{O}$  of Na component is in terms of  $\text{Na}_2\text{O}$ , and mol content of K component of  $\text{NK}_2\text{O}$  is in terms of  $\text{K}_2\text{O}$ .

The glaze layer of the spark plug of this composition is the same as the first and second compositions in that the Pb component is 1 mol % or less in terms of  $\text{PbO}$ . Accordingly, the Effect A can be obtained. While either or both of the Si and B components are contained, the amounts of the three components of Li, Na and K are adjusted to satisfy the above mentioned relationship, so that a new effect can be exhibited as follows.

(Effect F)

The alkaline metal component is inherently high in an ion conductivity, and serves to lower the insulating properties in a vitreous glaze layer. On the other hand, the Si or B components form the glass skeleton, and if their contents are appropriately determined, dimensions of skeletal meshes are made convenient for blocking the ion conductivity of the alkaline metal, and the favorable insulating properties can be secured. As the Si or B components easily form the skeleton, they act to reduce the fluidity when baking the glaze, but if containing the alkaline metal component in the above mentioned range, the fluidity when baking the glaze is increased by lowering of the melting point owing to eutectic reaction and avoidance of complex anion owing to interaction of S ion and O ion.

Herein, since the K component has a larger atomic weight than Na and Li as mentioned above, in case of setting a total containing amount of the alkaline metal components in the same mol %, the K component does not exhibit the improved effect of the fluidity as the Na and Li components do, but comparing with Na and Li (in particular Li), since an ionic mobility in the vitreous glaze layer is relatively small, the K component has a property difficult to decrease the insulating properties of the glaze layer though increasing the containing amount. On the other hand, since the Li component is small in the atomic weight, the improved effect of the fluidity is larger than that of the K component, but as the ionic mobility is high, an excessive addition is apt to cause the insulating properties of the glaze layer to decrease. However, being different from the K component, the Li component has a property to reduce the thermal expansion coefficient.

Accordingly, the insulating property of the glazing layer can be effectively prevented from decreasing by making the most amount of the K component, and the fluidity when baking the glaze can be secured by mixing the Li component with a containing amount next to that of the K component, and at the same time it is possible to suppress the increase of the thermal expansion coefficient of the glaze layer by mixing the K component, enabling to agree with the thermal expansion coefficient of a substrate alumina. A trend of decreasing the insulating property by adding the Li component can be effectively restrained by an effect of joint addition (later mentioned) of the three components where the Na component is less than K and Li. As a result, an ideal composition of the glaze is realized which is high in the insulating property, rich in the fluidity when baking the glaze, and small in the difference of the thermal expansion coefficient from that of alumina as the insulator composing ceramics. That is, the second problem of the invention is solved.

The glaze layer to be used with the third composition may have a composition corresponding to the glaze composition of the above first and/or second glaze.

Explanation will be made to the critical meaning of the containing range of each glaze layer in the above mentioned spark plug compositions. If the total amount in terms of oxides of one or two kinds or more of Mo, W, Ni, Co, Fe and Mn (called as "fluidity improving transition metal component" hereafter) is less than 0.5 mol %, there will be probably a case of not always providing an effect of improving the fluidity when baking the glaze for easily obtaining a smooth glaze layer. On the other hand, if exceeding 5 mol %, there will be probably a case of being difficult or impossible to bake the glaze owing to too much heightening of the softening point of the glaze.

As a problem when the containing amount of the fluidity improving transition metal component is excessive, such a case may be taken up that not intentioned coloring appears in the glaze layer. For example, visual information such as letters, figures or product numbers are printed with color glazes on external appearances of the insulators for specifying producers and others, and if the colors of the glaze layer is too thick, it might be difficult to read out the printed visual information. As another realistic problem, there is a case that tint changing resulted from alternation in the glaze composition is seen to purchasers as "unreasonable alternation in familiar colors in external appearance", so that an inconvenience occurs that products could not always be quickly accepted because of a resistant feeling thereto.

The insulator forming a substrate of the glaze layer comprises alumina based ceramics taking white, and in view of preventing or restraining coloration, it is desirable that the coloration in an observed external appearance of the glaze layer formed in the insulator is adjusted to be 0 to 6 in chroma Cs and 7.5 to 10 in lightness Vs, for example, the amount of the above transition metal component is adjusted. If the chroma exceeds 6, the gray or blackish coloration is easily distinguished. In either way, there appears a problem that an impression of "apparent coloration" cannot be wiped out. The chroma Cs is preferably 8 to 10, more preferably 9 to 10. In the present specification, a measuring method of the lightness Vs and the chroma Cs adopts the method specified in "4.3 A Measuring Method of Reflected Objects" of "4. Spectral Colorimetry" in the "A Measuring Method of Colors" of JIS-Z8721. As a simple method, the lightness and the chroma can be known through visual comparisons with standard color chart prepared according to JIS-Z8721.

That the effect of improving the fluidity when baking the glaze is especially remarkable is exhibited by W next to Mo and Fe. For example, it is possible that all the essential transition metal components are made Mo, Fe or W. For more heightening the effect of improving the fluidity when baking the glaze, it is preferable that Mo is 50 mol % or more of the essential transition metals.

Next, desirably, the total amount of the alkaline metal components is 5 to 10 mol %. In case of being less than 5 mol %, the softening point of the glaze goes up, baking of the glaze might be probably impossible. In case of being more than 10 mol %, the insulating property probably goes down, and an anti-flashover might be spoiled. The containing amount of the alkaline metal components is preferably 5 to 8 mol %. With respect to the alkaline metal components, not depending on one kind, but adding in joint two kinds or more selected from Na, K and Li, the insulating property of the glaze layer is more effectively restrained from lowering. As a result, the amount of the alkaline metal components can be increased without decreasing the insulating property,

consequently it is possible to concurrently attain the two purposes of securing the fluidity when baking the glaze and the anti-flashover (so-called alkaline joint addition effect).

Of the alkaline components of Na, K and Li, it is desirable to determine the rate of the K component in terms of oxide to be  $0.4 \leq K/(Na+K+Li) \leq 0.8$ .

Thereby, the effect of increasing the insulating property is more heightened. But if the value of  $K/(Na+K+Li)$  is less than 0.4, this effect is probably insufficient.

On the other hand, a reason for the value of  $K/(Na+K+Li)$  to be 0.8 or less is for securing the fluidity when baking the glaze, which means that the other alkaline metal components than K is added in joint in a range of the rest balance being 0.2 or more (0.6 or less). It is more preferable that the value of  $K/(Na+K+Li)$  is adjusted to be 0.5 to 0.7.

Further, in the alkaline metal components, preferably the Li component is contained if feasible for exhibiting the joint-addition of alkaline components so as to improve the insulating property, adjusting the thermal expansion coefficient of the glaze layer, securing the fluidity when baking the glaze, and heightening mechanical strength.

It is desirable that the Li component in mol % in terms of the oxide to be determined to be

$$0.2 \leq Li/(Na+K+Li) \leq 0.5.$$

If Li is less than 0.2, the thermal expansion coefficient is too large in comparison with that of the substrate alumina, and consequently defects such as crazing easily occur, so that it might be insufficient to secure a finish of the baked glaze surface. In contrast, if Li is more than 0.5, as an Li ion is relatively high in mobility among the alkaline metal ions, bad influences are probably given to the insulating property. It is better that values of  $Li/(Na+K+Li)$  are desirably adjusted to range 0.3 to 0.45. For more heightening the insulating property by the joint addition of the alkaline metal components, it is possible to mix other alkaline metal components following the third component as Na in a range where the electric conductivity is not spoiled by excessive joint-addition of the total amount of the alkaline metal components. In particular desirably, it is good to contain all the three components of Na, K and Li.

With respect to the Si component, being less than 25 mol %, it is often difficult to secure a sufficient insulating performance. Being more than 45 mol %, it is often difficult to bake the glaze. The Si containing amount should be more preferably 30 to 40 mol %.

If the B containing amount is less than 20 mol %, the softening point of the glaze goes up, and the baking of the glaze will be difficult. On the other hand, being more than 40 mol %, a glaze crimping is easily caused. Depending on containing amounts of other components, such apprehensions might occur as a devitrification the glaze layer, the lowering of the insulating property, or inconsequence of the thermal expansion coefficient in relation with the substrate. It is good to determine the B containing amount to range 25 to 35 mol % if possible.

If the Zn containing amount is less than 5 mol %, the thermal expansion coefficient of the glaze layer is too large, defects such as crazing are easily occur in the glaze layer. As the Zn component acts to lower the softening point of the glaze, if it is short, the baking of the glaze will be difficult. Being more than 25 mol %, opacity easily occurs in the glaze layer due to the devitrification. It is good that the Zn containing amount to determine 10 to 20 mol %.

The Ba and Sr components contribute to heightening of the insulating property of the glaze layer and is effective to increasing of the strength. If the total amount is less than 0.5

mol %, the insulating property of the glaze layer goes down, and the anti-flashover might be spoiled. Being more than 20 mol %, the thermal expansion coefficient of the glaze layer is too high, defects such as crazing are easily occur in the glaze layer. From the viewpoint of heightening the insulating property and adjusting the thermal expansion coefficient, the total amount of Ba and Sr is desirably determined to be 0.5 to 1.0 mol %. Either or both of the Ba and Sr component may be contained, but the Ba component is advantageously cheaper in a cost of a raw material.

The Ba and Sr components may exist in forms other than oxides in the glaze depending on raw materials to be used. For example,  $BaSO_4$  is used as a source of the Ba component, an S component might be residual in the glaze layer. This sulfur component is concentrated nearly to the surface of the glaze layer when baking the glaze to lower the surface expansion of a melted glaze and to heighten a smoothness of a glaze layer to be obtained.

The total amount of the Zn and Ba and/or Sr components is desirably 8 to 30 mol % in terms of the above mentioned oxides. Being more than 30 mol %, the opacity will occur in the glaze layer. For example, the visual information such as letters, figures or product numbers are printed with color glazes on external appearances of the insulators for specifying producers and others, it might be difficult to read out the printed visual information owing to such as the opacity. Being less than 8 mol %, the softening point extremely goes up, the glaze baking is difficult and a bad external appearance is caused. Preferably, the total amount is 10 to 20 mol %.

The one or two kinds or more of the Al component of 1 to 10 mol % in terms of  $Al_2O_3$ , the Ca component of 1 to 10 mol % in terms of  $CaO$ , and the Mg component of 0.1 to 10 mol % in terms of  $MgO$  may be contained 1 to 15 mol % in total. The Al component is effective to restraining the devitrification, while the Ca and Mg components contribute to heightening of the insulating property of the glaze layer. In particular, the Ca component is next to the Ba or Zn components to be useful for improving the insulating property of the glaze layer. If the addition amount is less than each of the lower limits, the effect is insufficient, and if being more than the upper limit of each component or more than the upper limit of the total amount, it is difficult or impossible to bake the glaze by the extreme increase of the softening point of the glaze layer.

In the viewpoint of the thermal expansion coefficient, it is preferable that in case B is in terms of  $B_2O_3$  and Zn is in terms of  $ZnO$ , the total mol containing amount is  $N(B_2O_3 + ZnO)$ , and in case the alkaline earth metal component RE (RE is one or two kinds or more selected from Ba, Mg, Ca and Sr) is in terms of composition formula of  $REO$  and the alkaline metal component R (R is one or two kinds or more selected from Na, K and Li) is in terms of composition formula of  $R_2O$ , the total mol containing amount is  $N(REO + R_2O)$ , and preferable is to be

$$1.5 \leq N(B_2O_3 + ZnO)/N(REO + R_2O) \leq 3.0.$$

This denotes that  $B_2O_3$  and  $ZnO$  act to decrease the thermal expansion coefficient, while the alkaline earth metal oxide  $REO$  and the alkaline metal oxide  $R_2O$  act to increase the thermal expansion coefficient, so that it is possible to agree to the thermal expansion coefficient in relation with the substrate of alumina. As a result, the glaze layer can be prevented from appearances of defects such as crazing, cracking or peeling. If the above ranges are less than 1.5, the thermal expansion coefficient is too large in comparison with

that of the substrate alumina, and consequently defects such as crazing easily occur, so that it might be insufficient to secure the finish of the baked glaze surface. In contrast, being more than 3.0, the thermal expansion coefficient is too small in comparison with that of the substrate alumina, resulting in easily causing cracking, peeling or crimping in the glaze layer. For making these effects more remarkable, preferable is to be

$$1.7 \leq N(B_2O_3 + ZnO) / N(ReO + R_2O) \leq 2.5.$$

Auxiliary components of one or two kinds or more of Bi, Sn, Sb, P, Cu, Ce and Cr may be contained 5 mol % or less in total as Bi in terms of  $Bi_2O_3$ , Sn in terms of  $SnO_2$ , Sn in terms of  $Sb_2O_5$ , P in terms of  $P_2O_5$ , Cu in terms of  $CuO$ , Ce in terms of  $CeO_2$ , and Cr in terms of  $Cr_2O_3$ . These components may be positively added in response to purposes or often inevitably included as raw materials of the glaze (otherwise later mentioned clay minerals to be mixed when preparing a glaze slurry) or impurities (otherwise contaminants) from refractory materials in the melting procedure for producing glaze frit. Each of them heightens the fluidity when baking the glaze, restrains bubble formation in the glaze layer, or wraps adhered materials on the baked glaze surface so as to prevent abnormal projections Bi and Sb are especially effective.

In the composition of the spark plug of the invention, the respective components in the glaze are contained in the forms of oxides, and owing to factors forming amorphous and vitreous phases, existing forms as oxides cannot be often identified. In such cases, if the containing amounts of components at values in terms of oxides fall in the above mentioned ranges, it is regarded that they belong to the ranges of the invention.

The containing amounts of the respective components in the glaze layer formed on the insulator can be identified by use of known micro-analyzing methods such as EPMA (electronic probe micro-analysis) or XPS (X-ray photoelectron spectroscopy). For example, if using EPMA, either of a wavelength dispersion system and an energy dispersion system is sufficient for measuring characteristic X-ray. Further, there is a method where the glaze layer is peeled from the insulator and is subjected to a chemical analysis or a gas analysis for identifying the composition.

The spark plug having the glaze layer of the invention maybe composed by furnishing, in a through hole of the insulator, an axially shaped terminal metal fixture as one body with the center electrode or holding a conductive binding layer in relation therewith, said metal fixture being separate from a center electrode. In this case, the whole of the spark plug is kept at around  $500^\circ C.$ , and an electric conductivity is made between the terminal metal fixture and a metal shell, enabling to measure the insulating resistant value. For securing an insulating endurance at high temperatures, it is desirable that the insulating resistant value is secured  $200 M\Omega$  or higher, desirably  $400 M\Omega$  or higher so as to prevent the flashover.

FIGS. 8A to 8D show one example of measuring system. That is, DC constant voltage source (e.g., source voltage 1000 V) is connected to the side of a terminal metal 13 of the spark plug 100, while at the same time, the side of the metal shell 1 is grounded, and a current is passed under a condition where the spark plug 100 disposed in a heating oven is heated at  $500^\circ C.$  For example, imagining that a current value  $Im$  is measured by use of a current measuring resistance (resistance value  $Rm$ ) at the voltage  $VS$ , an insulation resistance value  $Rx$  to be measured can be obtained as  $(VS/Im) - Rm$  (in the drawing, the current value

$Im$  is measured by output of a differential amplifier for amplifying voltage difference at both ends of the current measuring resistance).

The insulator may comprise the alumina insulating material containing the Al component 85 to 98 mol % in terms of  $Al_2O_3$ . Preferably, the glaze has an average thermal expansion coefficient of  $5 \times 10^{-6}/^\circ C.$  to  $8.5 \times 10^{-6}/^\circ C.$  at the temperature ranging 20 to  $350^\circ C.$  Being less than this lower limit, defects such as cracking or glaze skipping easily happen in the glaze layer. On the other hand, being more than the upper limit, defects such as crazing are easy to happen in the glaze layer. The thermal expansion coefficient more preferably ranges  $6 \times 10^{-6}/^\circ C.$  to  $8 \times 10^{-6}/^\circ C.$

The thermal expansion coefficient of the glaze layer is assumed in such ways that samples are cut out from a vitreous glaze bulk body prepared by mixing and melting raw materials such that almost the same composition as the glaze layer is realized, and values measured by a known dilatometer method. The thermal expansion coefficient of the glaze layer on the insulator can be measured by use of, e.g., a laser interferometer or an interatomic force microscope.

The insulator is formed with a projection part in an outer circumferential direction at an axially central position thereof. Taking, as a front side, a side directing toward the front end of the center electrode in the axial direction, a cylindrical face is shaped in the outer circumferential face at the base portion of the insulator main body in the neighborhood of a rear side opposite the projection part. In this case, the outer circumferential face at the base portion is covered with the glaze layer formed with the film thickness ranging 7 to  $50 \mu m$ .

In automobile engines, such a practice is broadly adopted that the spark plug is attached to engine electric equipment system by means of rubber caps, and for heightening the anti-flashover, important is the adherence between the insulator and the inside of the rubber cap. The inventors made earnest studies and found that, in the leadless glaze of borosilicate glass or alkaline borosilicate, it is important to adjust thickness of the glaze layer for obtaining a smooth surface of the baked glaze, and as the outer circumference of the base portion of the insulator main body particularly requires the adherence with the rubber cap, unless appropriate adjustment is made to the film thickness, as sufficient anti-flashover cannot be secured. Therefore, in the insulator having the leadless glaze layer of the above mentioned composition of the spark plug according to the third invention, if the film thickness of the glaze layer covering the outer circumference of the base portion of the insulator is set in the range of the above numerical values, the adherence with the baked glaze face and the rubber cap may be heightened, and in turn the anti-flashover may be improved without lowering the insulating property of the glaze layer.

If the thickness of the glaze layer at said base portion of the insulator is less than  $7 \mu m$ , the leadless glaze of the above mentioned composition is difficult to form the smooth baked surface, so that the adherence with the baked glaze face and the rubber cap is spoiled and the anti-flashover is made insufficient. But if the thickness of the glaze layer is more than  $50 \mu m$ , a cross sectional area of the electric conductivity increases, the leadless glaze of the above mentioned composition is difficult to secure the insulating property, probably resulting in lowering of the anti-flashover.

For uniforming the thickness of the glaze layer or controlling excessively (or partially) thick glaze layers, it is useful to add Ti, Zr or Hf as mentioned above.

## 11

The spark plug of the invention can be produced by a production method comprising

- a step of preparing glaze powders in which the raw material powders are mixed at a predetermined ratio, the mixture is heated 1000 to 1500° C. and melted, the melted material is rapidly cooled, vitrified and ground into powder;
- a step of piling the glaze powder on the surface of an insulator to form a glaze powder layer; and
- a step of heating the insulator, thereby to bake the glaze powder layer on the surface of the insulator.

The powdered raw material of each component includes not only an oxide thereof (sufficient with complex oxide) but also other inorganic materials such as hydroxide, carbonate, chloride, sulfate, nitrate, or phosphate. These inorganic materials should be those of capable of being converted to corresponding oxides by heating and melting. The rapidly cooling can be carried out by throwing the melt into a water or atomizing the melt onto the surface of a cooling roll for obtaining flakes.

The glaze powder is dispersed into the water or solvent, so that it can be used as a glaze slurry. For example, if coating the glaze slurry onto the insulator surface to dry it, the piled layer of the glaze powder can be formed as a coated layer of the glaze slurry. By the way, as the method of coating the glaze slurry on the insulator surface, if adopting a method of spraying from an atomizing nozzle onto the insulator surface, the piled layer in uniform thickness of the glaze powder can be easily formed and an adjustment of the coated thickness is easy.

The glaze slurry can contain an adequate amount of a clay mineral or an organic binder for heightening a shape retention of the piled layer of the glaze powder. As the clay mineral, those composed of mainly aluminosilicate hydrates can be applied, for example, those composed of mainly one or two kinds or more of allophane, imogolite, hisingerite, smectite, kaolinite, halloysite, montmorillonite, vermiculite, and dolomite (or mixtures thereof) can be used. In relation with the oxide components, in addition to  $\text{SiO}_2$  and  $\text{Al}_2\text{O}_3$ , those mainly containing one or two kinds or more of  $\text{Fe}_2\text{O}_3$ ,  $\text{TiO}_2$ ,  $\text{CaO}$ ,  $\text{MgO}$ ,  $\text{Na}_2\text{O}$  and  $\text{K}_2\text{O}$  can be used.

The spark plug of the invention is constructed of an insulator having a through-hole formed in the axial direction thereof, a terminal metal fixture fitted in one end of the through-hole, and a center electrode fitted in the other end. The terminal metal fixture and the center electrode are electrically connected via an electrically conductive sintered body mainly comprising a mixture of a glass and a conductive material (e.g., a conductive glass seal or a resistor). The spark plug having such a structure can be made by a process including the following steps.

An assembly step: a step of assembling a structure comprising the insulator having the through-hole, the terminal metal fixture fitted in one end of the through-hole, the center electrode fitted in the other end, and a filled layer formed between the terminal metal fixture and the center electrode, which filled layer comprises the glass powder and the conductive material powder.

A glaze baking step: a step of heating the assembled structure formed with the piled layer of the glaze powder on the surface of the insulator at temperature ranging 800 to 950° C. to bake the piled layer of the glaze powder on the surface of the insulator so as to form a glaze layer, and at the same time softening the glass powder in the filled layer.

A pressing step: a step of bringing the center electrode and the terminal metal fixture relatively close within the through-hole, thereby pressing the filled layer between the

## 12

center electrode and the terminal metal fixture into the electrically conductive sintered body.

In this case, the terminal metal fixture and the center electrode are electrically connected by the electrically conductive sintered body to concurrently seal the gap between the inside of the through-hole and the terminal metal fixture and the center electrode. Therefore, the glaze baking step also serves as a glass sealing step. This process is efficient in that the glass sealing and the glaze baking are performed simultaneously. Since the above mentioned glaze allows the baking temperature to be lower to 800 to 950° C., the center electrode and the terminal metal fixture hardly suffer from bad production owing to oxidation so that the yield of the spark plug is heightened. It is also sufficient that the baking glaze step is preceded to the glass sealing step.

The softening point of the glaze layer is preferably adjusted to range, e.g., 520 to 700° C. When the softening point is higher than 700° C., the baking temperature above 950° C. will be required to carry out both baking and glass sealing, which may accelerate oxidation of the center electrode and the terminal metal fixture. When the softening point is lower than 520° C., the glaze baking temperature should be set lower than 800° C. In this case, the glass used in the conductive sintered body must have a low softening point in order to secure a satisfactory glass seal. As a result, when an accomplished spark plug is used for a long time in a relatively high temperature environment, the glass in the conductive sintered body is liable to denaturalization, and where, for example, the conductive sintered body comprises a resistor, the denaturalization of the glass tends to result in deterioration of the performance such as a life under load. Incidentally, the softening point of the glaze is adjusted at temperature range of 520 to 620° C.

The softening point of the glaze layer is a value measured by performing a differential thermal analysis on the glaze layer peeled off from the insulator and heated, and it is obtained as a temperature of a peak appearing next to a first endothermic peak (that the second endothermic peak) which is indicative of a sag point. The softening point of the glaze layer formed in the surface of the insulator can be also estimated from a value obtained with a glass sample which is prepared by compounding raw materials so as to give substantially the same composition as the glaze layer under analysis, melting the composition and rapidly cooling.

Modes for carrying out the invention will be explained with reference to the accompanying drawings. FIG. 1 shows an example of the spark plug of the first structure according to the invention. The spark plug 100 has a cylindrical metal shell 1, an insulator 2 fitted in the inside of the metal shell 1 with its tip 21 projecting from the front end of the metal shell 1, a center electrode 3 disposed inside the insulator 2 with its ignition part 31 formed at the tip thereof, and a ground electrode 4 with its one end welded to the metal shell 1 and the other end bent inward such that a side of this end may face the tip of the center electrode 3. The ground electrode 4 has an ignition part 32 which faces the ignition part 31 to make a spark gap g between the facing ignition parts.

The metal shell 1 is formed to be cylindrical of such as a low carbon steel. It has a thread 7 therearound for screwing the spark plug 100 into an engine block (not shown). Symbol 1e is a hexagonal nut portion over which a tool such as a spanner or wrench fits to fasten the metal shell 1.

The insulator 2 has a through-hole 6 penetrating in the axial direction. A terminal fixture 13 is fixed in one end of the through-hole 6, and the center electrode 3 is fixed in the other end. A resistor 15 is disposed in the through-hole 6

between the terminal metal fixture 13 and the center electrode 3. The resistor 15 is connected at both ends thereof to the center electrode 3 and the terminal metal fixture 13 via the conductive glass seal layers 16 and 17, respectively. The resistor 15 and the conductive glass seal layers 16, 17 constitute the conductive sintered body. The resistor 15 is formed by heating and pressing a mixed powder of the glass powder and the conductive material powder (and, if desired, ceramic powder other than the glass) in a later mentioned glass sealing step. The resistor 15 may be omitted, and the terminal metal fixture 13 and the center electrode 3 may be directly connected by one seal layer of the conductive glass seal.

The insulator 2 has the through-hole 6 in its axial direction for fitting the center electrode 3, and is formed as a whole with an insulating material as follows. That is, the insulating material is mainly composed of an alumina ceramic sintered body having an Al content of 85 to 98 mol % (preferably 90 to 98 mol %) in terms of  $\text{Al}_2\text{O}_3$ .

The specific components other than Al are exemplified as follows.

Si component: 1.50 to 5.00 mol % in terms of  $\text{SiO}_2$ ;

Ca component: 1.20 to 4.00 mol % in terms of  $\text{CaO}$ ;

Mg component: 0.05 to 0.17 mol % in terms of  $\text{MgO}$ ;

Ba component: 0.15 to 0.50 mol % in terms of  $\text{BaO}$ ; and

B component: 0.15 to 0.50 mol % in terms of  $\text{B}_2\text{O}_3$ .

The insulator 2 has a projection 2e projecting outwardly, e.g., flange-like on its periphery at the middle part in the axial direction, a rear portion 2b whose outer diameter is smaller than the projecting portion 2e, a first front portion 2g in front of the projecting portion 2e, whose outer diameter is smaller than the projecting portion 2e, and a second front portion 2i in front of the first front portion 2g, whose outer diameter is smaller than the first front portion 2g. The rear end part of the rear portion 2b has its periphery corrugated to form corrugations 2c. The first front portion 2g is almost cylindrical, while the second front portion 2i is tapered toward the tip 21.

On the other hand, the center electrode 3 has a smaller diameter than that of the resistor 15. The through-hole 6 of the insulator 2 is divided into a first portion 6a (front portion) having a circular cross section in which the center electrode 3 is fitted and a second portion 6b (rear portion) having a circular cross section with a larger diameter than that of the first portion 6a. The terminal metal fixture 13 and the resistor 15 are disposed in the second portion 6b, and the center electrode 3 is inserted in the first portion 6a. The center electrode 3 has an outward projection 3c around its periphery near the rear end thereof, with which it is fixed to the electrode. A first portion 6a and a second portion 6b of the through-hole 6 are connected each other in the first front portion 2g in FIG. 3A, and at the connecting part, a projection receiving face 6c is tapered or rounded for receiving the projection 3c for fixing the center electrode 3.

The first front portion 2g and the second front portion 2i of the insulator 2 connect at a connecting part 2h, where a level difference is formed on the outer surface of the insulator 2. The metal shell 1 has a projection icon its inner wall at the position meeting the connecting part 2h so that the connecting part 2h fits the projection 1c via a gasket ring 63 thereby to prevent slipping in the axial direction. A gasket ring 62 is disposed between the inner wall of the metal shell 1 and the outer side of the insulator 2 at the rear of the flange-like projecting portion 2e, and a gasket ring 60 is provided in the rear of the gasket ring 62. The space between the two gaskets 60 and 62 is filled with a filler 61 such as

talc. The insulator 2 is inserted into the metal shell 1 toward the front end thereof, and under this condition, the rear opening edge of the metal shell 1 is pressed inward the gasket 60 to form a sealing lip 1d, and the metal shell 1 is secured to the insulator 2.

FIGS. 3A and 3B show practical examples of the insulator 2. The ranges of dimensions of these insulators are as follows.

Total length L1: 30 to 75 mm;

Length L2 of the first front portion 2g: 0 to 30 mm (exclusive of the connecting part 2f to the projecting portion 2e and inclusive of the connecting part 2h to the second front portion 2i);

Length L3 of the second front portion 2i: 2 to 27 mm;

Outer diameter D1 of the rear portion 2b: 9 to 13 mm; Outer diameter D2 of the projecting portion 2e: 11 to 16 mm;

Outer diameter D3 of the first front portion 2g: 5 to 11 mm; Outer base diameter D4 of the second front portion 2i: 3 to 8 mm;

Outer tip diameter D5 of the second front portion 2i (where the outer circumference at the tip is rounded or beveled, the outer diameter is measured at the base of the rounded or beveled part in a cross section containing the center axial line O): 2.5 to 7 mm;

Inner diameter D6 of the second portion 6b of the through-hole 6: 2 to 5 mm;

Inner diameter D7 of the first portion 6a of the through-hole 6: 1 to 3.5 mm;

Thickness t1 of the first front portion 2g: 0.5 to 4.5 mm; Thickness t2 at the base of the second front portion 2i (the thickness in the direction perpendicular to the center axial line O): 0.3 to 3.5 mm;

Thickness t3 at the tip of the second front portion 2i (the thickness in the direction perpendicular to the center axial line O; where the outer circumference at the tip is rounded or beveled, the thickness is measured at the base of the rounded or beveled part in a cross section containing the center axial line O): 0.2 to 3 mm; and

Average thickness tA ((2+t3)/2) of the second front portion 2i: 0.25 to 3.25 mm.

In FIG. 1, a length LQ of the portion 2k of the insulator 2 which projects over the rear end of the metal shell 1, is 23 to 27 mm (e.g., about 25 mm). In a vertical cross section containing the center axial line O of the insulator 2 on the outer contour of the projecting portion 2k of the insulator 2, the length LP of the portion 2k as measured along the profile of the insulator 2 is 26 to 32 mm (e.g., about 29 mm) starting from a position corresponding to the rear end of the metal shell 1, through the surface of the corrugations 2c, to the rear end of the insulator 2.

The insulator 2 shown in FIG. 3A has the following dimensions L1=ca. 60 mm, L2=ca. 10 mm, L3=ca. 14 mm, D1=ca. 11 mm, D2=ca. 13 mm, D3=ca. 7.3 mm, D4=5.3 mm, D5=4.3 mm, D6=3.9 mm, D7=2.6 mm, t1=3.3 mm, t2=1.4 mm, t3=0.9 mm, and tA=1.15 mm.

The insulator 2 shown in FIG. 3B is designed to have slightly larger outer diameters in its first and second front portions 2g and 2i than in the example shown in FIG. 3A. It has the following dimensions L1=ca. 60 mm, L2=ca. 10 mm, L3=ca. 14 mm, D1=ca. 11 mm, D2=ca. 13 mm, D3=ca. 9.2 mm, D4=6.9 mm, D5=5.1 mm, D6=3.9 mm, D7=2.7 mm, t1=3.3 mm, t2=2.1 mm, t3=1.2 mm, and tA=1.65 mm.

As shown in FIG. 2, the glaze layer 2d is formed on the outer surface of the insulator 2, more specifically, on the outer peripheral surface of the rear portion 2b inclusive of the corrugated part 2c. The glaze layer 2d has a thickness of

7 to 150  $\mu\text{m}$ , preferably 10 to 50  $\mu\text{m}$ . As shown in FIG. 1, the glaze layer 2d formed on the rear portion 2b extends in the front direction farther from the rear end of the metal shell 1 to a predetermined length, while the rear side extends till the rear end edge of the rear portion 2b.

The glaze layer 2d has anyone of the compositions explained in the columns of the means for solving the problems, works and effects. As the critical meaning in the composition range of each component has been referred to in detail, no repetition will be made herein. The thickness  $\text{tg}$  (average value) of the glaze layer 2d on the outer circumference of the base of the rear portion 2b (the cylindrical and non-corrugated outer circumference part 2c projecting downward from the metal shell 1) is 7 to 50  $\mu\text{m}$ . The corrugations 2c may be omitted. In this case, the average thickness of the glaze layer 2d on the area from the rear end of the metal shell 1 up to 50% of the projecting length LQ of the main part 1b is taken as  $\text{tg}$ .

The ground electrode 4 and the core 3a of the center electrode are made of an Ni alloy. The core 3a of the center electrode 3 is buried inside with a core 3b comprising Cu or Cu alloy for accelerating heat dissipation. An ignition part 31 and an opposite ignition part 32 are mainly made of a noble metal alloy based on one or two kinds or more of Ir, Pt and Rh. The core 3a of the center electrode 3 is reduced in diameter at a front end and is formed to be flat at the front face, to which a disk made of the alloy composing the ignition part is superposed, and the periphery of the joint is welded by a laser welding, electron beam welding, or resistance welding to form a welded part W, thereby constructing the ignition part 31. The opposite ignition part 32 positions a tip to the ground electrode 4 at the position facing the ignition part 31, and the periphery of the joint is welded to form a similar welded part W along an outer edge part. The tips are prepared by a molten metal comprising alloying components at a predetermined ratio or forming and sintering an alloy powder or a mixed powder of metals having a predetermined ratio. At least one of the ignition part 31 and the opposite ignition part 32 may be omitted.

The spark plug 100 can be produced as follows. In preparing the insulator 2, an alumina powder is mixed with raw material powders of a Si component, Ca component, Mg component, Ba component, and B component in such a mixing ratio as to give the aforementioned composition after sintering, and the mixed powder is mixed with a prescribed amount of a binder (e.g., PVA) and a water to prepare a slurry. The raw material powders include, for example,  $\text{SiO}_2$  powder as the Si component,  $\text{CaCO}_3$  powder as the Ca component,  $\text{MgO}$  powder as the Mg component,  $\text{BaCO}_3$  as the Ba component, and  $\text{H}_3\text{PO}_4$  as to the B component.  $\text{H}_3\text{BO}_3$  may be added in the form of a solution.

A slurry is spray-dried into granules for forming a base, and the base forming granules are rubber-pressed into a pressed body a prototype of the insulator. The formed body is processed on an outer side by grinding to the contour of the insulator 2 shown in FIG. 1, and then baked 1400 to 1600°C. to obtain the insulator 2.

The glaze slurry is prepared as follows.

Raw material powders as sources of Si, B, Zn, Ba, and alkaline components (Na, K, Li) (for example,  $\text{SiO}_2$  powder for the Si component,  $\text{H}_3\text{PO}_4$  powder for the B component,  $\text{ZnO}$  powder for the Zn component,  $\text{BaCO}_3$  powder for the Ba component,  $\text{Na}_2\text{CO}_3$  powder for the Na component,  $\text{K}_2\text{CO}_3$  powder for the K component, and  $\text{Li}_2\text{CO}_3$  powder for the Li component) are mixed for obtaining a predetermined composition. The mixed powder is heated and melted 1000 to 1500°C., and thrown into the water to rapidly cool

for vitrification, followed by grinding to prepare a glaze fritz. The glaze fritz is mixed with appropriate amounts of clay mineral, such as kaolin or gairome clay, and organic binder, and the water is added thereto to prepare the glaze slurry.

As shown in FIG. 7, the glaze slurry S is sprayed from a nozzle N to coat a requisite surface of the insulator 2, thereby to form a coated layer 2d' of the glaze slurry as the piled layer of the glaze powder.

The center electrode 3 and the terminal metal fixture 13 are fitted in the insulator 2 formed with the glaze slurry coated layer 2d' as well as the resistor 15 and the electrically conductive glass seal layers 16, 17 are formed as follows. As shown in FIG. 8A, the center electrode 3 is inserted into the first portion 6a of the through-hole 6. Then a conductive glass powder H is filled in the through-hole 6 as shown in FIG. 8B. The powder H is preliminary compressed by pressing a press bar 28 into the through-hole 6 to form a first conductive glass powder layer 26. A raw material powder for a resistor composition is filled and preliminary compressed in the same manner, so that, as shown in FIG. 8D, the first conductive glass powder 26, the resistor composition powder layer 25 and a second conductive glass powder layer 27 are laminated from the center electrode 3 (lower side) into the through-hole 6.

An assembled structure PA is formed where the terminal metal fixture 13 is disposed from the upper part into the through-hole 6 as shown in FIG. 9A. The assembled structure PA is put into a heating oven and heated at a predetermined temperature of 800 to 950°C. being above the glass softening point, and then the terminal metal fixture 13 is pressed into the through-hole 6 from aside opposite to the center electrode 3 so as to press the superposed layers 25 to 27 in the axial direction. Thereby, as seen in FIG. 9B, the layers are each compressed and sintered to become a conductive glass seal layer 16, a resistor 15, and a conductive glass seal layer 17 (the above is the glass sealing step).

If the softening point of the glaze powder contained in the glaze slurry coated layer 2d' is set to be 600 to 700°C., the layer 2d' can be baked as shown in FIGS. 9A and 9B, at the same time as the heating in the above glass sealing step, into the glaze layer 2d. Since the heating temperature of the glass sealing step is selected from the relatively low temperature of 800 to 950°C., oxidation to surfaces of the center electrode 3 and the terminal metal fixture 13 can be made less.

If a burner type gas furnace is used as the heating oven (which also serves as the glaze baking oven), a heating atmosphere contains relatively much steam as a combustion product. If the glaze composition containing the B component 40 mol % or less is used, the fluidity when baking the glaze can be secured even in such an atmosphere, and it is possible to form the glaze layer of smooth and homogeneous substance and excellent in the insulation.

After the glass sealing step, the metal shell 1, the ground electrode 4 and others are fitted on the structure PA to complete spark plug 100 shown in FIG. 1. The spark plug 100 is screwed into an engine block using the thread 7 thereof and used as a spark source to ignite an air/fuel mixture supplied to a combustion chamber. A high-tension cable or an ignition coil is connected to the spark plug 100 by means of a rubber cap RC (comprising, e.g., silicone rubber). The rubber cap RC has a smaller hole diameter than the outer diameter D1 (FIG. 3) of the rear portion 2b by about 0.5 to 1.0 mm. The rear portion 2b is pressed into the rubber cap while elastically expanding the hole until it is covered therewith to its base.

As a result, the rubber cap **RC** comes into close contact with the outer surface of the rear portion **2b** to function as an insulating cover for preventing flashover.

By the way, the spark plug of the invention is not limited to the type shown in FIG. 1, but for example as shown in FIG. 4, the tip of the ground electrode **4** is made to face the side of the center electrode **3** to form an ignition gap **g**. Further, as shown in FIG. 5, a semi-planar discharge type spark plug is also useful where the front end of the insulator **2** is advanced between the side of the center electrode **3** and the front end of the ground electrode **4**.

### EXAMPLES

For confirmation of the effects according to the invention, the following experiments were carried out.  
(Experiment 1)

The insulator **2** was made as follows. Alumina powder (alumina content: 95 mol %; Na content (as  $\text{Na}_2\text{O}$ ): 0.1 mol %; average particle size: 3.0  $\mu\text{m}$ ) was mixed at a predetermined mixing ratio with  $\text{SiO}_2$  (purity: 99.5%; average particle size: 1.5  $\mu\text{m}$ ),  $\text{CaCO}_3$  (purity: 99.9%; average particle size: 2.0  $\mu\text{m}$ ),  $\text{MgO}$  (purity: 99.5%; average particle size: 2  $\mu\text{m}$ )  $\text{BaCO}_3$  (purity: 99.5%; average particle size: 1.5  $\mu\text{m}$ ),  $\text{H}_3\text{BO}_3$  (purity: 99.0%; average particle size 1.5  $\mu\text{m}$ ), and  $\text{ZnO}$  (purity: 99.5%, average particle size: 2.0  $\mu\text{m}$ ). To 100 parts by weight of the resulting mixed powder were added 3 parts by weight of PVA as a hydrophilic binder and 103 parts by weight of water, and the mixture was kneaded to prepare a slurry.

The resulting slurry was spray-dried into spherical granules, which were sieved to obtain fraction of 50 to 100  $\mu\text{m}$ . The granules were formed under a pressure of 50 MPa by a known rubber-pressing method. The outer surface of the formed body was machined with the grinder into a predetermined figure and baked at 1550° C. to obtain the insulator **2**. The X-ray fluorescence analysis revealed that the insulator **2** had the following composition.

Al component (as  $\text{Al}_2\text{O}_3$ ): 94.9 mol %;  
Si component (as  $\text{SiO}_2$ ): 2.4 mol %;  
Ca component (as  $\text{CaO}$ ): 1.9 mol %;  
Mg component (as  $\text{MgO}$ ): 0.1 mol %;  
Ba component (as  $\text{BaO}$ ): 0.4 mol %; and  
B component (as  $\text{B}_2\text{O}_3$ ): 0.3 mol %.

The insulator **2** shown in FIG. 3A has the following dimensions.  $L1=\text{ca.}60\text{ mm}$ ,  $L2=\text{ca.}8\text{ mm}$ ,  $L3=\text{ca.}14\text{ mm}$ ,  $D1=\text{ca.}10\text{ mm}$ ,  $D2=\text{ca.}13\text{ mm}$ ,  $D3=\text{ca.}7\text{ mm}$ ,  $D4=5.5\text{ mm}$ ,  $D5=4.5\text{ mm}$ ,  $D6=4\text{ mm}$ ,  $D7=2.6\text{ mm}$ ,  $t1=1.5\text{ mm}$ ,  $t2=1.45\text{ mm}$ ,  $t3=1.25\text{ mm}$ , and  $tA=1.35\text{ mm}$ . In FIG. 1, a length  $LQ$  of the portion **2k** of the insulator **2** which projects over the rear end of the metal shell **1**, is 25 mm. In a vertical cross section containing the center axial line **O** of the insulator **2** on the outer contour of the projecting portion **2k** of the insulator **2**, the length  $LP$  of the portion **2k** as measured along the profile of the insulator **2** is 29 mm, starting from a position corresponding to the rear end of the metal shell **1**, through the surface of the corrugations **2c**, to the rear end of the insulator **2**.

$\text{SiO}_2$  powder (purity: 99.5%),  $\text{Al}_2\text{O}_3$  powder (purity: 99.5%),  $\text{H}_3\text{BO}_3$  powder (purity: 98.5%),  $\text{Na}_2\text{CO}_3$  powder (purity: 99.5%),  $\text{K}_2\text{CO}_3$  powder (purity: 99%),  $\text{Li}_2\text{CO}_3$  powder (purity: 99%),  $\text{BaSO}_4$  powder (purity: 99.5%),  $\text{SrCO}_3$  powder (purity: 99%),  $\text{ZnO}$  powder (purity: 99.5%),  $\text{MoO}_3$  powder (purity: 99%),  $\text{Fe}_2\text{O}_3$  powder (purity: 99%),  $\text{WO}_3$  powder (purity: 99%),  $\text{Ni}_3\text{O}_4$  powder (purity: 99%),  $\text{Co}_3\text{O}_4$  powder (purity: 99%),  $\text{MnO}_2$  powder (purity: 99%),  $\text{CaO}$  powder (purity: 99.5%),  $\text{TiO}_2$  powder (purity: 99.5%),

$\text{ZrO}_2$  powder (purity: 99.5%),  $\text{HfO}_2$  powder (purity: 99%),  $\text{MgO}$  powder (purity: 99.5%),  $\text{Sb}_2\text{O}_5$  powder (purity: 99%),  $\text{Bi}_2\text{O}_3$  powder (purity: 99%),  $\text{SnO}_2$  powder (purity: 99.5%),  $\text{P}_2\text{O}_5$  powder (purity: 99%),  $\text{CuO}$  powder (purity: 99%),  $\text{CeO}_2$  powder (purity: 99.5%), and  $\text{Cr}_2\text{O}_3$  powder (purity: 99.5%) were mixed. The mixture was melted 1000 to 1500° C., and the melt was poured into the water and rapidly cooled for vitrification, followed by grinding in an alumina pot mill to powder of 50  $\mu\text{m}$  or smaller. Three parts by weight of New Zealand kaolin and 2 parts by weight of PVA as an organic binder were mixed into 100 parts by weight of the glaze powder, and the mixture was kneaded with 100 parts by weight of the water to prepare the glaze slurry.

The glaze slurry was sprayed on the insulator **2** from the spray nozzle as illustrated in FIG. 7, and dried to form the coated layer **2d** of the glaze slurry having a coated thickness of about 100  $\mu\text{m}$ . Several kinds of the spark plug **100** were produced by using the insulator **2** through the process explained with reference to FIGS. 11 to 12. The outer diameter of the thread **7** was 14 mm. The resistor **15** was made of the mixed powder consisting of  $\text{B}_2\text{O}_3$ — $\text{SiO}_2$ — $\text{BaO}$ — $\text{LiO}_2$  glass powder,  $\text{ZrO}_2$  powder, carbon black powder,  $\text{TiO}_2$  powder, and metallic Al powder. The electrically conductive glass seal layers **16**, **17** were made of the mixed powder consisting of  $\text{B}_2\text{O}_3$ — $\text{SiO}_2$ — $\text{Na}_2\text{O}$  glass powder, Cu powder, Fe powder, and Fe—B powder. The heating temperature for the glass sealing, i.e., the glaze baking temperature was set at 900° C.

On the other hand, such glaze samples were produced which were not pulverized but solidified in block. The block-like sample was confirmed by the X-ray diffraction to be a vitrified (amorphous) state.

The experiments were performed as follows.

#### (1) Chemical Composition Analysis

The X-ray fluorescence analysis was conducted. The analyzed value per each sample (in terms of oxide) was shown in Tables 1 to 6. The analytical results obtained by EPMA on the glaze layer **2d** formed on the insulator were almost in agreement with the results measured with the block-like samples.

#### (2) Thermal Expansion Coefficient

The specimen of 5 mm×5 mm×5 mm was cut out from the block-like sample, and measured with the known dilatometer method at the temperature ranging 20 to 350° C. The same measurement was made at the same size of the specimen cut out from the insulator **2**. As a result, the value was  $73 \times 10^{-7}/^\circ\text{C}$ .

#### (3) Softening Point

The powder sample weighing 50 mg was subjected to the differential thermal analysis, and the heating was measured from a room temperature. The second endothermic peak was taken as the softening point.

With respect to the respective spark plugs, the insulation resistance at 500° C. was evaluated at the applied voltage 1000V through the process explained with reference to FIGS. 8A to 8D. Further, the appearance of the glaze layer **2d** formed on the insulator **2** was visually observed. The film thickness of the glaze layer on the outer circumference of the base edge part of the insulator was measured in the cross section by the SEM observation. In judgements of the outer appearance of the glaze layer, no abnormality seen in luster and transparency is excellent (OO), and slight crimping or devitrification, though being within an allowable range is good (O). Apparent abnormality is specifically shown within the column as to kinds of abnormalities. The above mentioned results are shown in Tables 1 to 6.

TABLE 1

| Com.<br>(mol %)                | 1    | 2    | 3    | 4    | 5    | 6    | 7    |
|--------------------------------|------|------|------|------|------|------|------|
| SiO <sub>2</sub>               | 36.0 | 36.0 | 36.0 | 36.0 | 36.0 | 36.0 | 36.0 |
| Al <sub>2</sub> O <sub>3</sub> | 2.0  | 2.0  | 2.0  | 2.0  | 2.0  | 2.0  | 2.0  |
| B <sub>2</sub> O <sub>3</sub>  | 28.0 | 28.0 | 28.0 | 28.0 | 28.0 | 28.0 | 28.0 |
| Na <sub>2</sub> O              | 1.0  | 1.0  | 1.0  | 1.0  | 1.0  | 1.0  | 1.0  |
| K <sub>2</sub> O               | 4.5  | 4.5  | 4.5  | 4.5  | 4.5  | 4.5  | 4.5  |
| Li <sub>2</sub> O              | 2.0  | 2.0  | 2.0  | 2.0  | 2.0  | 2.0  | 2.0  |
| BaO                            | 4.5  | 4.5  | 2.5  | —    | 4.5  | 4.5  | 4.5  |
| SrO                            | —    | —    | 2.0  | 4.5  | —    | —    | —    |
| ZnO                            | 16.0 | 16.0 | 16.0 | 16.0 | 16.0 | 16.0 | 16.0 |
| MoO <sub>3</sub>               | 1.0  | 1.0  | 1.0  | 1.0  | —    | —    | —    |
| Fe <sub>2</sub> O <sub>3</sub> | —    | —    | —    | —    | —    | 1.0  | —    |
| WO <sub>3</sub>                | —    | —    | —    | —    | —    | 1.0  | —    |
| Ni <sub>3</sub> O <sub>4</sub> | —    | —    | —    | —    | —    | —    | 0.5  |
| Co <sub>3</sub> O <sub>4</sub> | —    | —    | —    | —    | —    | —    | 0.5  |
| MnO <sub>2</sub>               | —    | —    | —    | —    | —    | —    | —    |
| CaO                            | 4.0  | 5.0  | 4.0  | 4.0  | 4.0  | 4.0  | 4.0  |
| ZrO <sub>2</sub>               | 1.0  | —    | 1.0  | 1.0  | 1.0  | 1.0  | 1.0  |
| TiO <sub>2</sub>               | —    | —    | —    | —    | —    | —    | —    |
| HfO <sub>2</sub>               | —    | —    | —    | —    | —    | —    | —    |
| MgO                            | —    | —    | —    | —    | —    | —    | —    |
| Sb <sub>2</sub> O <sub>5</sub> | —    | —    | —    | —    | —    | —    | —    |
| Bi <sub>2</sub> O <sub>3</sub> | —    | —    | —    | —    | —    | —    | —    |

TABLE 1-continued

| 5  | SnO <sub>2</sub>                            | —    | —    | —    | —    | —    | —    |
|----|---------------------------------------------|------|------|------|------|------|------|
|    | P <sub>2</sub> O <sub>5</sub>               | —    | —    | —    | —    | —    | —    |
|    | CuO                                         | —    | —    | —    | —    | —    | —    |
|    | CeO <sub>2</sub>                            | —    | —    | —    | —    | —    | —    |
|    | Cr <sub>2</sub> O <sub>3</sub>              | —    | —    | —    | —    | —    | —    |
| 10 | Total                                       | 100  | 100  | 100  | 100  | 100  | 100  |
|    | K/(Na + Li + K)                             | 0.60 | 0.60 | 0.60 | 0.60 | 0.60 | 0.60 |
|    | Li/(Na + Li + K)                            | 0.27 | 0.27 | 0.27 | 0.27 | 0.27 | 0.27 |
|    | ZnO + BaO + SrO                             | 20.5 | 20.5 | 20.5 | 20.5 | 20.5 | 20.5 |
|    | Al <sub>2</sub> O <sub>3</sub> + CaO + MgO  | 6.0  | 7.0  | 6.0  | 6.0  | 6.0  | 6.0  |
|    | Coefficient of                              | 7.0  | 7.0  | 7.0  | 7.0  | 7.0  | 7.0  |
| 15 | Thermal expansion<br>( $\times 10^{-6}$ )   | —    | —    | —    | —    | —    | —    |
|    | Softening point (° C.)                      | 570  | 570  | 570  | 570  | 570  | 570  |
|    | Insulation<br>resistance at 500° C.<br>(MΩ) | 800  | 400  | 900  | 800  | 800  | 800  |
| 20 | Appearance                                  | ○○   | ○○   | ○○   | ○○   | ○○   | ○○   |
|    | Film thickness of<br>Glaze layer (μm)       | 40   | 60   | 20   | 40   | 30   | 40   |

Com:Composition

\*shows "outside" of the invention

TABLE 2

| Com.<br>(mol %)                | SiO <sub>2</sub>                            | 8    | 9    | 10   | 11   | 12   | 13   | 14   |
|--------------------------------|---------------------------------------------|------|------|------|------|------|------|------|
| Al <sub>2</sub> O <sub>3</sub> | 2.0                                         | 2.0  | 2.0  | —    | 2.0  | 2.0  | 2.0  | 2.0  |
| B <sub>2</sub> O <sub>3</sub>  | 28.0                                        | 28.0 | 28.0 | 28.0 | 28.0 | 28.0 | 28.0 | 28.0 |
| Na <sub>2</sub> O              | 1.0                                         | 2.5  | 3.5  | 3.5  | 2.0  | 0.5  | 0.5  | 0.5  |
| K <sub>2</sub> O               | 4.5                                         | 2.5  | —    | —    | 4.5  | 2.5  | 2.5  | 2.5  |
| Li <sub>2</sub> O              | 2.0                                         | 2.5  | 3.0  | 3.0  | 1.0  | 4.5  | 4.5  | 4.5  |
| BaO                            | 4.5                                         | 4.5  | 4.5  | 4.5  | 4.5  | 4.5  | 4.5  | 4.5  |
| SrO                            | —                                           | —    | —    | —    | —    | —    | —    | —    |
| ZnO                            | 16.0                                        | 16.0 | 16.0 | 16.0 | 16.0 | 16.0 | 16.0 | 16.0 |
| MoO <sub>3</sub>               | —                                           | 1.0  | 1.0  | 1.0  | 1.0  | 1.0  | 1.0  | 1.0  |
| Fe <sub>2</sub> O <sub>3</sub> | —                                           | —    | —    | —    | —    | —    | —    | —    |
| WO <sub>3</sub>                | —                                           | —    | —    | —    | —    | —    | —    | —    |
| Ni <sub>3</sub> O <sub>4</sub> | —                                           | —    | —    | —    | —    | —    | —    | —    |
| Co <sub>3</sub> O <sub>4</sub> | —                                           | —    | —    | —    | —    | —    | —    | —    |
| MnO <sub>2</sub>               | 1.0                                         | —    | —    | —    | —    | —    | —    | —    |
| CaO                            | 4.0                                         | 4.0  | 4.0  | 4.0  | 4.0  | 4.0  | 4.0  | 5.0  |
| ZrO <sub>2</sub>               | 1.0                                         | 1.0  | 1.5  | 1.5  | 1.0  | 1.0  | 1.0  | —    |
| TiO <sub>2</sub>               | —                                           | —    | 0.5  | 0.5  | —    | —    | —    | —    |
| HfO <sub>2</sub>               | —                                           | —    | —    | —    | —    | —    | —    | —    |
| MgO                            | —                                           | —    | —    | —    | —    | —    | —    | —    |
| Sb <sub>2</sub> O <sub>5</sub> | —                                           | —    | —    | —    | —    | —    | —    | —    |
| Bi <sub>2</sub> O <sub>3</sub> | —                                           | —    | —    | —    | —    | —    | —    | —    |
| SnO <sub>2</sub>               | —                                           | —    | —    | —    | —    | —    | —    | —    |
| P <sub>2</sub> O <sub>5</sub>  | —                                           | —    | —    | —    | —    | —    | —    | —    |
| CuO                            | —                                           | —    | —    | —    | —    | —    | —    | —    |
| CeO <sub>2</sub>               | —                                           | —    | —    | —    | —    | —    | —    | —    |
| Cr <sub>2</sub> O <sub>3</sub> | —                                           | —    | —    | —    | —    | —    | —    | —    |
| 100                            | Total                                       | 100  | 100  | 100  | 100  | 100  | 100  | 100  |
|                                | K/(Na + Li + K)                             | 0.60 | 0.33 | 0.00 | 0.00 | 0.60 | 0.33 | 0.33 |
|                                | Li/(Na + Li + K)                            | 0.27 | 0.33 | 0.46 | 0.46 | 0.13 | 0.60 | 0.60 |
|                                | ZnO + BaO + SrO                             | 20.5 | 20.5 | 20.5 | 20.5 | 20.5 | 20.5 | 20.5 |
|                                | Al <sub>2</sub> O <sub>3</sub> + CaO + MgO  | 6.0  | 6.0  | 6.0  | 4.0  | 6.0  | 6.0  | 7.0  |
|                                | Coefficient of                              | 7.0  | 6.8  | 7.0  | 6.9  | 7.2  | 6.6  | 6.6  |
| 15                             | Thermal expansion<br>( $\times 10^{-6}$ )   | —    | —    | —    | —    | —    | —    | —    |
|                                | Softening point (° C.)                      | 570  | 560  | 550  | 545  | 575  | 550  | 545  |
|                                | Insulation<br>resistance at 500° C.<br>(MΩ) | 700  | 450  | 350  | 350  | 900  | 300  | 100  |
| 20                             | Appearance                                  | ○○   | ○○   | ○    | ○    | ○    | ○○   | ○○   |
|                                | Film thickness of<br>glaze layer (μm)       | 50   | 30   | 20   | 20   | 50   | 20   | 60   |

Com.: Composition

\*shows "outside" of the invention

TABLE 3

| Com.<br>(mol %)                | 15   | 16   | 17*  | 18*  | 19   | 20   | 21   |
|--------------------------------|------|------|------|------|------|------|------|
| SiO <sub>2</sub>               | 38.0 | 36.0 | 30.0 | 36.0 | 36.0 | 37.0 | 37.0 |
| Al <sub>2</sub> O <sub>3</sub> | —    | 2.0  | 2.0  | 2.0  | 2.0  | 2.0  | 2.0  |
| B <sub>2</sub> O <sub>3</sub>  | 28.0 | 28.0 | 33.0 | 30.0 | 25.0 | 28.0 | 30.0 |
| Na <sub>2</sub> O              | 0.5  | 1.0  | 4.0  | 0.5  | 1.0  | 1.0  | 1.0  |
| K <sub>2</sub> O               | 2.5  | 6.5  | 2.0  | 1.0  | 4.5  | 4.5  | 4.5  |
| Li <sub>2</sub> O              | 4.5  | 2.0  | 5.5  | 3.0  | 2.0  | 2.0  | 2.0  |
| BaO                            | 4.5  | 7.5  | 4.5  | 4.5  | 2.0  | 7.0  | 7.0  |
| SrO                            | —    | —    | —    | —    | —    | —    | —    |
| ZnO                            | 16.0 | 11.0 | 16.0 | 16.0 | 23.0 | 7.0  | 9.0  |
| MoO <sub>3</sub>               | 1.0  | 1.0  | 1.0  | 1.5  | 0.5  | 2.0  | —    |
| Fe <sub>2</sub> O <sub>3</sub> | —    | —    | —    | —    | —    | —    | —    |
| WO <sub>3</sub>                | —    | —    | —    | —    | —    | —    | —    |
| Ni <sub>3</sub> O <sub>4</sub> | —    | —    | —    | —    | —    | —    | —    |
| Co <sub>3</sub> O <sub>4</sub> | —    | —    | —    | —    | —    | —    | —    |
| MnO <sub>2</sub>               | —    | —    | —    | —    | —    | —    | —    |
| CaO                            | 5.0  | 4.0  | —    | —    | 3.0  | 4.5  | 4.5  |
| ZrO <sub>2</sub>               | —    | 1.0  | 2.0  | 2.0  | 1.0  | 1.0  | —    |
| TiO <sub>2</sub>               | —    | —    | —    | —    | —    | 1.0  | —    |
| HfO <sub>2</sub>               | —    | —    | —    | —    | —    | —    | —    |
| MgO                            | —    | —    | —    | 3.5  | —    | 3.0  | 3.0  |
| Sb <sub>2</sub> O <sub>5</sub> | —    | —    | —    | —    | —    | —    | —    |
| Bi <sub>2</sub> O <sub>3</sub> | —    | —    | —    | —    | —    | —    | —    |
| SnO <sub>2</sub>               | —    | —    | —    | —    | —    | —    | —    |
| P <sub>2</sub> O <sub>5</sub>  | —    | —    | —    | —    | —    | —    | —    |

TABLE 3-continued

| 5                                         | 15                                          | 16   | 17*  | 18*  | 19   | 20   | 21   |
|-------------------------------------------|---------------------------------------------|------|------|------|------|------|------|
| CuO                                       | —                                           | —    | —    | —    | —    | —    | —    |
| CeO                                       | —                                           | —    | —    | —    | —    | —    | —    |
| Cr <sub>2</sub> O <sub>3</sub>            | —                                           | —    | —    | —    | —    | —    | —    |
| 10                                        | Total                                       | 100  | 100  | 100  | 100  | 100  | 100  |
| K/(Na + Li + K)                           | 0.33                                        | 0.68 | 0.17 | 0.22 | 0.60 | 0.60 | 0.60 |
| Li/(Na + Li + K)                          | 0.60                                        | 0.21 | 0.48 | 0.67 | 0.27 | 0.27 | 0.27 |
| ZnO + BaO + SrO                           | 20.5                                        | 18.5 | 20.5 | 20.5 | 25.0 | 14.0 | 16.0 |
| 15                                        | Al <sub>2</sub> O <sub>3</sub> + CaO + MgO  | 5.0  | 6.0  | 2.0  | 5.5  | 5.0  | 9.5  |
| Coefficient of                            | 6.5                                         | 8.0  | 8.5  | 6.4  | 6.5  | 7.7  | 7.7  |
| Thermal expansion<br>( $\times 10^{-6}$ ) |                                             |      |      |      |      |      |      |
| Softening point (° C.)                    | 540                                         | 555  | 540  | 590  | 550  | 590  | 590  |
| 20                                        | Insulation<br>resistance at 500° C.<br>(MΩ) | 100  | 550  | 200  | 1500 | 450  | 1200 |
| Appearance                                | ○                                           | ○○   | A    | B    | ○○   | ○○   | ○○   |
| 25                                        | Film thickness of<br>glaze layer (μm)       | 60   | 40   | 30   | 40   | 50   | 65   |

Com:Composition A:Crazing B:Insufficient glaze-melting

\*shows "outside" of the invention

TABLE 4

|                 | 22                             | 23*  | 24*  | 25   | 26   | 27   | 28   |
|-----------------|--------------------------------|------|------|------|------|------|------|
| Com.<br>(mol %) | SiO <sub>2</sub>               | 39.0 | 30.0 | 35.0 | 35.0 | 35.0 | 35.0 |
|                 | Al <sub>2</sub> O <sub>3</sub> | —    | 1.5  | 2.0  | 2.0  | 2.0  | 2.0  |
|                 | B <sub>2</sub> O <sub>3</sub>  | 30.0 | 26.0 | 22.0 | 27.0 | 27.0 | 27.0 |
|                 | Na <sub>2</sub> O              | 1.0  | 2.0  | 4.5  | 1.0  | 1.0  | 1.0  |
|                 | K <sub>2</sub> O               | 4.5  | 1.0  | 2.0  | 4.5  | 4.5  | 4.5  |
|                 | Li <sub>2</sub> O              | 2.0  | 4.5  | 1.0  | 2.0  | 2.0  | 2.0  |
|                 | BaO                            | 7.0  | 3.0  | 20.0 | 13.0 | 13.0 | 13.0 |
|                 | SrO                            | —    | —    | —    | —    | —    | —    |
|                 | ZnO                            | 9.0  | 30.0 | 11.0 | 10.0 | 10.0 | 10.0 |
|                 | MoO <sub>3</sub>               | —    | 1.0  | 1.0  | 1.0  | 1.0  | 1.0  |
|                 | Fe <sub>2</sub> O <sub>3</sub> | —    | —    | 0.5  | —    | —    | —    |
|                 | WO <sub>3</sub>                | —    | —    | —    | —    | —    | —    |
|                 | Ni <sub>3</sub> O <sub>4</sub> | —    | —    | —    | —    | —    | —    |
|                 | Co <sub>3</sub> O <sub>4</sub> | —    | —    | —    | —    | —    | —    |
|                 | MnO <sub>2</sub>               | —    | —    | —    | —    | —    | —    |
|                 | CaO                            | 4.5  | —    | —    | 2.0  | 2.0  | 2.0  |
|                 | ZrO <sub>2</sub>               | —    | —    | 1.0  | 2.0  | 2.0  | 2.0  |
|                 | TiO <sub>2</sub>               | —    | 1.0  | —    | —    | —    | —    |
|                 | HfO <sub>2</sub>               | —    | —    | —    | —    | —    | —    |
|                 | MgO                            | 3.0  | —    | —    | —    | —    | —    |
|                 | Sb <sub>2</sub> O <sub>5</sub> | —    | —    | —    | 0.5  | —    | —    |
|                 | Bi <sub>2</sub> O <sub>3</sub> | —    | —    | —    | —    | 0.5  | —    |
|                 | SnO <sub>2</sub>               | —    | —    | —    | —    | —    | 0.5  |
|                 | P <sub>2</sub> O <sub>5</sub>  | —    | —    | —    | —    | —    | 0.5  |
|                 | CuO                            | —    | —    | —    | —    | —    | —    |
|                 | CeO <sub>2</sub>               | —    | —    | —    | —    | —    | —    |
|                 | Cr <sub>2</sub> O <sub>3</sub> | —    | —    | —    | —    | —    | —    |

|                                            |      |      |      |      |      |      |      |
|--------------------------------------------|------|------|------|------|------|------|------|
| Total                                      | 100  | 100  | 100  | 100  | 100  | 100  | 100  |
| K/(Na + Li + K)                            | 0.60 | 0.13 | 0.27 | 0.60 | 0.60 | 0.60 | 0.60 |
| Li/(Na + Li + K)                           | 0.27 | 0.60 | 0.13 | 0.27 | 0.27 | 0.27 | 0.27 |
| ZnO + BaO + SrO                            | 16.0 | 33.0 | 31.0 | 23.0 | 23.0 | 23.0 | 23.0 |
| Al <sub>2</sub> O <sub>3</sub> + CaO + MgO | 7.5  | 1.5  | 2.0  | 4.0  | 4.0  | 4.0  | 4.0  |

TABLE 4-continued

|                                                          | 22  | 23* | 24*  | 25  | 26  | 27   | 28  |
|----------------------------------------------------------|-----|-----|------|-----|-----|------|-----|
| Coefficient of thermal expansion ( $\times 10^{-6}$ )    | 7.6 | 6.0 | 8.7  | 7.9 | 7.9 | 7.9  | 7.9 |
| Softening point ( $^{\circ}$ C.)                         | 585 | 530 | 560  | 560 | 550 | 565  | 565 |
| Insulation resistance at 500 $^{\circ}$ C. (M $\Omega$ ) | 400 | 350 | 1000 | 900 | 900 | 1000 | 800 |
| Appearance                                               | ○   | D   | A    | ○○  | ○○  | ○○   | ○○  |
| Film thickness of glaze layer ( $\mu$ m)                 | 65  | 50  | 30   | 40  | 20  | 20   | 50  |

Com.: Composition

A: Crazing

D: Devitrification

\*shows "outside" of the invention

TABLE 5

|                                                          | 29   | 30   | 31   | 32*  | 33*  | 34   | 35   |
|----------------------------------------------------------|------|------|------|------|------|------|------|
| Com. SiO <sub>2</sub> (mol %)                            | 35.0 | 35.0 | 35.0 | 36.0 | 36.0 | 36.0 | 28.0 |
| Al <sub>2</sub> O <sub>3</sub>                           | 2.0  | 2.0  | 2.0  | 2.0  | 2.0  | 2.0  | 2.0  |
| B <sub>2</sub> O <sub>3</sub>                            | 27.0 | 27.0 | 27.0 | 28.0 | 27.0 | 28.0 | 33.5 |
| Na <sub>2</sub> O                                        | 1.0  | 1.0  | 1.0  | 4.5  | 4.5  | —    | 2.0  |
| K <sub>2</sub> O                                         | 4.5  | 4.5  | 4.5  | 2.0  | 2.0  | —    | 4.5  |
| Li <sub>2</sub> O                                        | 2.0  | 2.0  | 2.0  | 1.0  | 1.0  | 7.5  | 1.0  |
| BaO                                                      | 13.0 | 13.0 | 13.0 | 4.5  | 4.5  | 4.5  | 10.0 |
| SrO                                                      | —    | —    | —    | —    | —    | —    | —    |
| ZnO                                                      | 10.0 | 10.0 | 10.0 | 16.0 | 12.0 | 16.0 | 16.0 |
| MoO <sub>3</sub>                                         | 1.0  | 1.0  | 1.0  | —    | 4.0  | 1.0  | 1.0  |
| Fe <sub>2</sub> O <sub>3</sub>                           | —    | —    | —    | —    | 2.0  | 0.5  | —    |
| WO <sub>3</sub>                                          | —    | —    | —    | —    | —    | —    | —    |
| Ni <sub>3</sub> O <sub>4</sub>                           | —    | —    | —    | —    | —    | —    | —    |
| Co <sub>3</sub> O <sub>4</sub>                           | —    | —    | —    | —    | —    | —    | —    |
| MnO <sub>2</sub>                                         | —    | —    | —    | —    | —    | —    | —    |
| CaO                                                      | 2.0  | 2.0  | 2.0  | 4.0  | 4.0  | —    | 1.0  |
| ZrO <sub>2</sub>                                         | 2.0  | 2.0  | 2.0  | 1.0  | 1.0  | —    | 1.0  |
| TiO <sub>2</sub>                                         | —    | —    | —    | —    | —    | —    | —    |
| HfO <sub>2</sub>                                         | —    | —    | —    | —    | —    | —    | —    |
| MgO                                                      | —    | —    | —    | —    | —    | 3.5  | —    |
| Sb <sub>2</sub> O <sub>5</sub>                           | —    | —    | —    | 1.0  | —    | 1.0  | —    |
| Bi <sub>2</sub> O <sub>3</sub>                           | —    | —    | —    | —    | —    | —    | —    |
| SnO <sub>2</sub>                                         | —    | —    | —    | —    | —    | —    | —    |
| P <sub>2</sub> O <sub>5</sub>                            | —    | —    | —    | —    | —    | —    | —    |
| CuO                                                      | 0.5  | —    | —    | —    | —    | —    | —    |
| CeO <sub>2</sub>                                         | —    | 0.5  | —    | —    | —    | —    | —    |
| Cr <sub>2</sub> O <sub>3</sub>                           | —    | —    | 0.5  | —    | —    | —    | —    |
| Total                                                    | 100  | 100  | 100  | 100  | 100  | 100  | 100  |
| K/(Na + Li + K)                                          | 0.60 | 0.60 | 0.60 | 0.27 | 0.27 | 0.00 | 0.60 |
| Li/(Na + Li + K)                                         | 0.27 | 0.27 | 0.27 | 0.13 | 0.13 | 1.00 | 0.13 |
| ZnO + BaO + SrO                                          | 23.0 | 23.0 | 23.0 | 20.5 | 16.5 | 20.5 | 26.0 |
| Al <sub>2</sub> O <sub>3</sub> + CaO + MgO               | 4.0  | 4.0  | 4.0  | 6.0  | 6.0  | 5.5  | 3.0  |
| Coefficient of thermal expansion ( $\times 10^{-6}$ )    | 7.9  | 7.9  | 7.9  | 7.2  | 7.2  | 6.4  | 7.5  |
| Softening point ( $^{\circ}$ C.)                         | 565  | 535  | 565  | 570  | 580  | 540  | 550  |
| Insulation resistance at 500 $^{\circ}$ C. (M $\Omega$ ) | 800  | 800  | 800  | 800  | 800  | 50   | 600  |
| Appearance                                               | ○○   | ○○   | ○○   | E*   | D*   | ○○   | ○○   |
| Film thickness of glaze layer ( $\mu$ m)                 | 40   | 20   | 10   | 30   | 30   | 80   | 40   |

Com.: Composition

D\*: Devitrification

E\*: Bubbling

\*shows "outside" of the invention

TABLE 6

|                                                       | 36*  | 37   | 38*  | 39*  | 40   | 41   | 42*  |
|-------------------------------------------------------|------|------|------|------|------|------|------|
| Com. (mol %)                                          |      |      |      |      |      |      |      |
| SiO <sub>2</sub>                                      | 20.0 | 40.0 | 48.0 | 38.0 | 38.0 | 38.0 | 30.0 |
| Al <sub>2</sub> O <sub>3</sub>                        | 4.0  | 1.0  | 1.0  | 2.0  | 2.0  | 2.0  | 1.0  |
| B <sub>2</sub> O <sub>3</sub>                         | 38.0 | 28.0 | 25.0 | 18.0 | 22.0 | 22.0 | 41.0 |
| Na <sub>2</sub> O                                     | 4.5  | 1.0  | 5.5  | 4.5  | 1.0  | 1.0  | 2.0  |
| K <sub>2</sub> O                                      | 2.0  | 5.0  | 3.0  | 2.0  | 4.5  | 4.5  | 4.5  |
| Li <sub>2</sub> O                                     | 1.0  | 3.0  | 1.0  | 1.0  | 2.0  | 2.0  | 1.0  |
| BaO                                                   | 5.5  | 4.5  | 4.5  | 7.5  | 6.5  | 6.5  | 4.5  |
| SrO                                                   | —    | —    | —    | —    | —    | —    | —    |
| ZnO                                                   | 16.0 | 15.0 | 10.0 | 16.0 | 16.0 | 16.0 | 12.0 |
| MoO <sub>3</sub>                                      | 1.0  | 1.0  | 1.0  | 1.0  | 1.0  | 1.0  | 1.0  |
| Fe <sub>2</sub> O <sub>3</sub>                        | —    | —    | —    | —    | —    | —    | —    |
| WO <sub>3</sub>                                       | —    | —    | —    | —    | —    | —    | —    |
| Ni <sub>3</sub> O <sub>4</sub>                        | —    | —    | —    | —    | —    | —    | —    |
| Co <sub>3</sub> O <sub>4</sub>                        | —    | —    | —    | —    | —    | —    | —    |
| MnO <sub>2</sub>                                      | —    | —    | —    | —    | —    | —    | —    |
| CaO                                                   | 4.0  | —    | —    | 4.0  | 4.0  | 4.0  | 2.0  |
| ZrO <sub>2</sub>                                      | 2.0  | 1.0  | 1.0  | 1.0  | 1.0  | —    | 1.0  |
| TiO <sub>2</sub>                                      | 2.0  | 0.5  | —    | 2.0  | 2.0  | 2.0  | —    |
| HfO <sub>2</sub>                                      | —    | —    | —    | —    | —    | 1.0  | —    |
| MgO                                                   | —    | —    | —    | 3.0  | —    | —    | —    |
| Sb <sub>2</sub> O <sub>5</sub>                        | —    | —    | —    | —    | —    | —    | —    |
| Bi <sub>2</sub> O <sub>3</sub>                        | —    | —    | —    | —    | —    | —    | —    |
| SnO <sub>2</sub>                                      | —    | —    | —    | —    | —    | —    | —    |
| P <sub>2</sub> O <sub>5</sub>                         | —    | —    | —    | —    | —    | —    | —    |
| CuO                                                   | —    | —    | —    | —    | —    | —    | —    |
| CeO <sub>2</sub>                                      | —    | —    | —    | —    | —    | —    | —    |
| Cr <sub>2</sub> O <sub>3</sub>                        | —    | —    | —    | —    | —    | —    | —    |
| Total                                                 | 100  | 100  | 100  | 100  | 100  | 100  | 100  |
| K/(Na + Li + K)                                       | 0.27 | 0.56 | 0.32 | 0.27 | 0.60 | 0.60 | 0.60 |
| Li/(Na + Li + K)                                      | 0.13 | 0.33 | 0.11 | 0.13 | 0.27 | 0.27 | 0.13 |
| ZnO + BaO + SrO                                       | 21.5 | 19.5 | 14.5 | 23.5 | 22.5 | 22.5 | 16.5 |
| Al <sub>2</sub> O <sub>3</sub> + CaO + MgO            | 8.0  | 1.0  | 1.0  | 9.0  | 6.0  | 6.0  | 3.0  |
| Coefficient of thermal expansion ( $\times 10^{-6}$ ) | 7.7  | 6.9  | 6.5  | 7.7  | 7.5  | 7.5  | 6.5  |
| Softening point (° C.)                                | 520  | 610  | 640  | 620  | 590  | 590  | 510  |
| Insulation resistance at 500° C. (MΩ)                 | 500  | 650  | 600  | 800  | 850  | 850  | 800  |
| Appearance                                            | F    | ○○   | B    | B    | ○○   | ○○   | G    |
| Film thickness of glaze layer (μm)                    | 30   | 30   | 20   | 40   | 40   | 10   | 50   |

Com.: Composition

B: Insufficient glaze-melting

F: Crimpings appear

G: Bubbles remain

\*shows "outside" of the invention

According to the results, depending on the compositions of the glaze of the invention, although no Pb is substantially contained, the glaze may be baked at relatively low temperatures, sufficient insulating properties are secured, and the outer appearance of the baked glaze faces are almost satisfied.

The entire disclosure of each and every foreign patent application from which the benefit of foreign priority has been claimed in the present application is incorporated herein by reference, as if fully set forth herein.

We claim:

1. A spark plug comprising:

a center electrode;

a metal shell; and

an alumina ceramic insulator disposed between the center electrode and the metal shell, wherein at least part of the surface of the insulator is covered with a glaze layer comprising oxides,

wherein the glaze layer comprises:

1 mol % or less of a Pb component in terms of PbO;

25 to 45 mol % of a Si component in terms of SiO<sub>2</sub>;20 to 40 mol % of a B component in terms of B<sub>2</sub>O<sub>3</sub>;

5 to 25 mol % of a Zn component in terms of ZnO;

0.5 to 15 mol % in total of at least one of Ba and Sr

components in terms of BaO and SrO, respectively;

5 to 10 mol % in total of at least one alkaline metal

component of Na, K and Li, in terms of Na<sub>2</sub>O, K<sub>2</sub>O,and Li<sub>2</sub>O, respectively,

0.5 to 5 mol % in total of at least one alkaline metal

component of Na, K and Li, in terms of Na<sub>2</sub>O, K<sub>2</sub>Oand Li<sub>2</sub>O respectively;

0.5 to 5 mole % in total of at least one of Mo, W, Ni,

Co, Fe and Mn in terms of MoO<sub>3</sub>, WO<sub>3</sub>, Ni<sub>3</sub>O<sub>4</sub>,Co<sub>3</sub>O<sub>4</sub>, Fe<sub>2</sub>O<sub>3</sub>, and MnO<sub>2</sub>, respectively,

wherein K has a highest content in the at least one

alkaline metal component in the glaze layer.

2. The sparkplug according to claim 1, wherein the glaze layer further comprises 0.5 to 5 mol % in total of at least one of Ti, Zr and Hf in terms of  $TiO_2$ ,  $ZrO_2$  and  $HfO_2$ , respectively.

3. A spark plug comprising:

a center electrode;

a metal shell; and

an alumina ceramic insulator disposed between the center electrode and the metal shell, wherein at least part of the surface of the insulator is covered with a glaze layer comprising oxides,

wherein the glaze layer comprises:

1 mol % or less of a Pb component in terms of  $PbO$ ;  
25 to 45 mol % of a Si component in terms of  $SiO_2$ ;  
20 to 40 mol % of a B component in terms of  $B_2O_3$ ;  
5 to 25 mol % of a Zn component in terms of  $ZnO$ ;  
0.5 to 15 mol % in total of at least one of Ba and Sr components in terms of  $BaO$  and  $SrO$ , respectively;  
5 to 10 mol % in total of at least one alkaline metal component of Na, K and Li, in terms of  $Na_2O$ ,  $K_2O$ , and  $Li_2O$ , respectively;  
0.5 to 5 mol % in total of at least one of Ti, Zr and Hf in terms of  $TiO_2$ ,  $ZrO_2$  and  $HfO_2$ , respectively; and  
0.5 to 5 mole % in total of at least one of Mo, W, Ni, Co, Fe and Mn in terms of  $MoO_3$ ,  $WO_3$ ,  $Ni_3O_4$ ,  $Co_3O_4$ ,  $Fe_2O_3$ , and  $MnO_2$ , respectively,

wherein the glaze layer comprises three components of Li, Na and K as the at least one alkaline metal components, and has a composition which satisfies the relationship of:

$$NNa_2O \leq NLi_2O \leq NK_2O$$

in which  $NLi_2O$  is a mol content of the Li component in terms of  $Li_2O$ ,  $NNa_2O$  is a mol content of the Na component in terms of  $Na_2O$ , and  $NK_2O$  is a mol content of the K component in terms of  $K_2O$ .

4. The spark plug according to any one of claims 1 and 3, wherein the glaze layer comprises three components of Li, Na and K as the at least one alkaline metal components, and has a composition which satisfies the relationship of:

$$NNa_2O \leq NLi_2O \leq NK_2O$$

in which  $NLi_2O$  is a mol content of the Li component in terms of  $Li_2O$ ,  $NNa_2O$  is a mol content of the Na component in terms of  $Na_2O$ , and  $NK_2O$  is a mol content of the K component in terms of  $K_2O$ .

5. A spark plug comprising:

a center electrode;

a metal shell; and

an alumina ceramic insulator disposed between the center electrode and the metal shell, wherein at least part of the surface of the insulator is covered with a glaze layer comprising oxides,

wherein the glaze layer comprises: 1 mol % or less of a Pb component in terms of  $PbO$ ; at least one of Si and B components as a glass skeleton structure; and three components of Li, Na and K as alkaline metal components, and the glaze layer has a composition which satisfies the relationship of:

$$NNa_2O \leq NLi_2O \leq NK_2O$$

in which  $NLi_2O$  is a mol content of the Li component in terms of  $Li_2O$ ,  $NNa_2O$  is a mol content of the Na component in terms of  $Na_2O$ , and  $NK_2O$  is a mol content of the K component in terms of  $K_2O$ .

6. The spark plug according to claim 1, wherein the glaze layer contains the K component and at least two alkaline metal components among the Li, Na and K components, and satisfies the relationship:  $0.4 < NK_2O/NR_2O < 0.8$  when the at least two alkaline metals are take as R,  $NR_2O$  is a total mol content of the at least two alkaline metals in terms of a composition formula  $R_2O$ , and  $NK_2O$  is a mol content of the K component in terms of  $K_2O$ .

7. The spark plug according to claim 3, wherein the glaze layer contains the K component and at least two alkaline metal components among the Li, Na and K components, and satisfies the relationship:  $0.4 < NK_2O/NR_2O < 0.8$  when the at least two alkaline metals are take as R,  $NR_2O$  is a total mol content of the at least two alkaline metals in terms of a composition formula  $R_2O$ , and  $NK_2O$  is a mol content of the K component in terms of  $K_2O$ .

8. The sparkplug according to claim 5, wherein the glaze layer contains the K component and at least two alkaline metal components among the Li, Na and K components, and satisfies the relationship:  $0.4 < NK_2O/NR_2O < 0.8$  when the at least two alkaline metals are take as R,  $NR_2O$  is a total mol content of the at least two alkaline metals in terms of a composition formula  $R_2O$ , and  $NK_2O$  is a mol content of the K component in terms of  $K_2O$ .

9. The spark plug according to claim 1, wherein the glaze layer contains the Li component and at least two alkaline metal components among the Li, Na and K components, and satisfies the relationship:  $0.2 < NLi_2O/NR_2O < 0.5$  when the at least two alkaline metals are take as R,  $NR_2O$  is a total mol content of the at least two alkaline metals in terms of a composition formula  $R_2O$ , and  $NLi_2O$  is a mol content of the Li component in terms of  $L_2O$ .

10. The spark plug according to claim 3, wherein the glaze layer contains the Li component and at least two alkaline metal components among the Li, Na and K components, and satisfies the relationship:  $0.2 < NLi_2O/NR_2O < 0.5$  when the at least two alkaline metals are take as R,  $NR_2O$  is a total mol content of the at least two alkaline metals in terms of a composition formula  $R_2O$ , and  $NLi_2O$  is a mol content of the Li component in terms of  $L_2O$ .

11. The spark plug according to claim 5, wherein the glaze layer contains the Li component and at least two alkaline metal components among the Li, Na and K components, and satisfies the relationship:  $0.2 < NLi_2O/NR_2O < 0.5$  when the at least two alkaline metals are take as R,  $NR_2O$  is a total mol content of the at least two alkaline metals in terms of a composition formula  $R_2O$ , and  $NLi_2O$  is a mol content of the Li component in terms of  $L_2O$ .

12. The spark plug according to claim 1, wherein the glaze layer contains the Zn component and the at least one of Ba and Sr components in an amount of 10 to 30 mol % in total in terms of  $ZnO$ ,  $BaO$  and  $SrO$ , respectively.

13. The spark plug according to claim 3, wherein the glaze layer contains the Zn component and the at least one of Ba and Sr components in an amount of 10 to 30 mol % in total in terms of  $ZnO$ ,  $BaO$  and  $SrO$ , respectively.

14. The spark plug according to claim 5, wherein the glaze layer contains the Zn component and the at least one of Ba and Sr components in an amount of 10 to 30 mol % in total in terms of  $ZnO$ ,  $BaO$  and  $SrO$ , respectively.

15. The spark plug according to claim 1, wherein the glaze layer further comprises 0.1 to 15 mol % in total of at least one of 0.1 to 10 mol % of an Al component in terms of  $Al_2O_3$ , 0.1 to 10 mol % of a Ca component in terms of  $CaO$ , and 0.1 to 10 mol % of a Mg component in terms of  $MgO$ .

16. The spark plug according to claim 3, wherein the glaze layer further comprises 0.1 to 15 mol % in total of at least

one of 0.1 to 10 mol % of an Al component in terms of  $\text{Al}_2\text{O}_3$ , 0.1 to 10 mol % of a Ca component in terms of  $\text{CaO}$ , and 0.1 to 10 mol % of a Mg component in terms of  $\text{MgO}$ .

17. The spark plug according to claim 5, wherein the glaze layer further comprises 0.1 to 15 mol % in total of at least one of 0.1 to 10 mol % of an Al component in terms of  $\text{Al}_2\text{O}_3$ , 0.1 to 10 mol % of a Ca component in terms of  $\text{CaO}$ , and 0.1 to 10 mol % of a Mg component in terms of  $\text{MgO}$ .

18. The spark plug according to claim 1, wherein the glaze layer further comprises 5 mol % or less in total of at least one of Bi, Sn, Sb, P, Cu, Ce and Cr in terms of  $\text{Bi}_2\text{O}_3$ ,  $\text{SnO}_2$ ,  $\text{Sb}_2\text{O}_5$ ,  $\text{P}_2\text{O}_5$ ,  $\text{CuO}$ ,  $\text{CeO}_2$  and  $\text{Cr}_2\text{O}_3$ , respectively.

19. The spark plug according to claim 3, wherein the glaze layer further comprises 5 mol % or less in total of at least one of Bi, Sn, Sb, P, Cu, Ce and Cr in terms of  $\text{Bi}_2\text{O}_3$ ,  $\text{SnO}_2$ ,  $\text{Sb}_2\text{O}_5$ ,  $\text{P}_2\text{O}_5$ ,  $\text{CuO}$ ,  $\text{CeO}_2$  and  $\text{Cr}_2\text{O}_3$ , respectively.

20. The spark plug according to claim 5, wherein the glaze layer further comprises 5 mol % or less in total of at least one of Bi, Sn, Sb, P, Cu, Ce and Cr in terms of  $\text{Bi}_2\text{O}_3$ ,  $\text{SnO}_2$ ,  $\text{Sb}_2\text{O}_5$ ,  $\text{P}_2\text{O}_5$ ,  $\text{CuO}$ ,  $\text{CeO}_2$  and  $\text{Cr}_2\text{O}_3$ , respectively.

21. The spark plug according to claim 1, wherein the insulator is formed with a projection part in an outer circumferential direction at an axially central position thereof,

taking, as a front side, a side directing toward the front end of the center electrode in the axial direction, a cylindrical face is shaped in the outer circumferential face at the base portion of the insulator main body in the neighborhood of a rear side opposite the projection part, and

the outer circumferential face at the base portion is covered with the glaze layer formed with a film thickness ranging 7 to 50  $\mu\text{m}$ .

22. The spark plug according to claim 3, wherein the insulator is formed with a projection part in an outer circumferential direction at an axially central position thereof,

taking, as a front side, a side directing toward the front end of the center electrode in the axial direction, a cylindrical face is shaped in the outer circumferential face at the base portion of the insulator main body in the neighborhood of a rear side opposite the projection part, and

the outer circumferential face at the base portion is covered with the glaze layer formed with a film thickness ranging 7 to 50  $\mu\text{m}$ .

23. The spark plug according to claim 5, wherein the insulator is formed with a projection part in an outer circumferential direction at an axially central position thereof,

taking, as a front side, a side directing toward the front end of the center electrode in the axial direction, a cylindrical face is shaped in the outer circumferential face at the base portion of the insulator main body in the neighborhood of a rear side opposite the projection part, and

the outer circumferential face at the base portion is covered with the glaze layer formed with a film thickness ranging 7 to 50  $\mu\text{m}$ .

24. The spark plug according to claim 1, which comprises one of: a terminal metal fixture and the center electrode as one body, in a through hole of the insulator; and a terminal metal fixture and the center electrode separated by a conductive bonding layer, and

an insulation resistance value is 400  $\text{M}\Omega$  or more, which is measured by keeping the whole of the spark plug at

about 500° C. and passing a current between the terminal metal fixture and the metal shell via the insulator.

25. The spark plug according to claim 3, which comprises one of: a terminal metal fixture and the center electrode as one body, in a through hole of the insulator; and a terminal metal fixture and the center electrode separated by a conductive bonding layer, and

an insulation resistant value is 400  $\text{M}\Omega$  or more, which is measured by keeping the whole of the spark plug at about 500° C. and passing a current between the terminal metal fixture and the metal shell via the insulator.

26. The spark plug according to claim 5, which comprises one of: a terminal metal fixture and the center electrode as one body, in a through hole of the insulator; and a terminal metal fixture and the center electrode separated by a conductive bonding layer, and

an insulation resistant value is 400  $\text{M}\Omega$  or more, which is measured by keeping the whole of the spark plug at about 500° C. and passing a current between the terminal metal fixture and the metal shell via the insulator.

27. The spark plug according to claim 1, wherein the insulator comprises an alumina insulating material containing 85 to 98 mol % of an Al component in terms of  $\text{Al}_2\text{O}_3$ , and the glaze layer has an average thermal expansion coefficient at the temperature ranging 20 to 350° C. of  $5 \times 10^{-6}/^\circ\text{C}$ . to  $8.5 \times 10^{-6}/^\circ\text{C}$ .

28. The spark plug according to claim 3, wherein the insulator comprises an alumina insulating material containing 85 to 98 mol % of an Al component in terms of  $\text{Al}_2\text{O}_3$ , and the glaze layer has an average thermal expansion coefficient at the temperature ranging 20 to 350° C. of  $5 \times 10^{-6}/^\circ\text{C}$ . to  $8.5 \times 10^{-6}/^\circ\text{C}$ .

29. The spark plug according to claim 5, wherein the insulator comprises an alumina insulating material containing 85 to 98 mol % of an Al component in terms of  $\text{Al}_2\text{O}_3$ , and the glaze layer has an average thermal expansion coefficient at the temperature ranging 20 to 350° C. of  $5 \times 10^{-6}/^\circ\text{C}$ . to  $8.5 \times 10^{-6}/^\circ\text{C}$ .

30. The spark plug according to claim 1, wherein the glaze layer has a softening point of 520 to 620° C.

31. The spark plug according to claim 3, wherein the glaze layer has a softening point of 520 to 620° C.

32. The spark plug according to claim 5, wherein the glaze layer has a softening point of 520 to 620° C.

33. A spark plug comprising:

a center electrode;  
a metal shell; and

an alumina ceramic insulator disposed between the center electrode and the metal shell, wherein at least part of the surface of the insulator is covered with a glaze layer comprising oxides,

wherein the glaze layer comprises:

1 mol % or less of a Pb component in terms of  $\text{PbO}$ ;  
25 to 45 mol % of a Si component in terms of  $\text{SiO}_2$ ;  
20 to 40 mol % of a B component in terms of  $\text{B}_2\text{O}_3$ ;  
5 to 25 mol % of a Zn component in terms of  $\text{ZnO}$ ;  
0.5 to 15 mol % in total of at least one of Ba and Sr components in terms of  $\text{BaG}$  and  $\text{SrO}$ , respectively;  
5 to 10 mol % in total of at least one alkaline metal component of Na, K and Li, in terms of  $\text{Na}_2\text{O}$ ,  $\text{K}_2\text{O}$ , and  $\text{Li}_2\text{O}$ , respectively, wherein K is essential; and  
0.5 to 5 mole % in total of at least one of Mo, W and Co in terms of  $\text{MoO}_3$ ,  $\text{WO}_3$  and  $\text{Co}_3\text{O}_4$ , respectively.

**31**

**34.** A spark plug comprising:  
a center electrode;  
a metal shell; and  
an alumina ceramic insulator disposed between the center <sup>5</sup> electrode and the metal shell, wherein at least part of the surface of the insulator is covered with a glaze layer comprising oxides,  
wherein the glaze layer comprises:  
1 mol % or less of a Pb component in terms of PbO; <sup>10</sup>  
25 to 45 mol % of a Si component in terms of SiO<sub>2</sub>;  
20 to 40 mol % of a B component in terms of B<sub>2</sub>O<sub>3</sub>;

**32**

5 to 25 mol % of a Zn component in terms of ZnO;  
0.5 to 15 mol % in total of at least one of Ba and Sr components in terms of BaO and SrO, respectively;  
5 to 10 mol % in total of at least one alkaline metal component of Na, K and Li, in terms of Na<sub>2</sub>O, K<sub>2</sub>O, and Li<sub>2</sub>O, respectively;  
0.5 to 5 mol % in total of at least one of Ti, Zr and Hf in terms of TiO<sub>2</sub>, ZrO<sub>2</sub> and HfO<sub>2</sub>, respectively; and  
0.5 to 5 mol % in total of at least one of Mo, W and Co in terms of MoO<sub>3</sub>, WO<sub>3</sub>, and Co<sub>3</sub>O<sub>4</sub>, respectively.

\* \* \* \* \*